



US006586171B1

(12) **United States Patent**  
Iwado

(10) **Patent No.:** US 6,586,171 B1  
(45) **Date of Patent:** Jul. 1, 2003

(54) **METHOD FOR DRYING COATING FILM IN MANUFACTURE OF THERMAL-DEVELOPABLE LIGHT-SENSITIVE MATERIAL**

(75) Inventor: **Junpei Iwado, Fujinomiya (JP)**

(73) Assignee: **Fuji Photo Film Co., Ltd., Kanagawa (JP)**

(\*) Notice: Subject to any disclaimer, the term of this patent is extended or adjusted under 35 U.S.C. 154(b) by 0 days.

(21) Appl. No.: **10/133,324**

(22) Filed: **Apr. 29, 2002**

(51) **Int. Cl.<sup>7</sup>** ..... G03C 1/74; G03C 1/498; F26B 13/20

(52) **U.S. Cl.** ..... 430/619; 430/531; 430/534; 430/935

(58) **Field of Search** ..... 430/619, 531, 430/935, 534; 34/370, 359, 418

(56)

**References Cited**

**U.S. PATENT DOCUMENTS**

6,423,487 B2 \* 7/2002 Naoi

**FOREIGN PATENT DOCUMENTS**

JP 2002-139814 \* 5/2002 ..... G03C1/74

\* cited by examiner

*Primary Examiner*—Thorl Chea

(57) **ABSTRACT**

Since a coating film is cured to some extent by the gelation of the coating film in the chilling-zone process and the first-stage drying in the PAC drying process, then, it is fully dried by the second-stage drying in the HAC drying process, liquid scattering from the surface of the coating film during drying can be prevented, even if the binder is difficult to cure as in the coating film for a thermal-developable light-sensitive material. Thereby, good coating film surface condition and good photographic performance can be obtained.

**18 Claims, 2 Drawing Sheets**



FIG.





**METHOD FOR DRYING COATING FILM IN  
MANUFACTURE OF  
THERMAL-DEVELOPABLE  
LIGHT-SENSITIVE MATERIAL**

**BACKGROUND OF THE INVENTION**

**1. Field of the Invention**

The present invention relates to a method for drying a coating film, and more specifically, to a method for drying a coating film for a thermal-developable light-sensitive material that uses an SBR (styrene-butadiene copolymer)-based binder and is difficult to be cured.

**2. Description of the Related Art**

In recent years, in the fields of medical diagnostic films and photoengraving films, the reduction of the quantities of treated waste liquids have strongly been demanded from the point of view of environmental preservation and space saving. In such a circumstance, technology related to thermal-developable light-sensitive materials has been desired for medical diagnostic films and photoengraving films that can be exposed efficiently using a laser image setter or a laser imager, and can form clear black images having high resolution and sharpness. The thermal-developable light-sensitive materials have advantages of providing a thermal developing system that needs no solvent-based chemicals for processing, can be used easily, and does not damage environment.

Coating liquids for light-sensitive materials can roughly be classified into coating liquids for silver halide photographic light-sensitive materials that use gelatin-based binders, and coating liquids for the above-described thermal-developable light-sensitive materials that use polymer-latex-based, for example, SBR (styrene-butadiene copolymer)-based binders. After coating a support with these coating liquids for light-sensitive materials to form a coating film, it is need to supply drying air to the coating film to dry the coating film.

However, the coating films using gelatin-based binders have characteristics of being cured easily; while the coating films using polymer-latex-based, for example, SBR (styrene-butadiene copolymer)-based binders have characteristics of being difficult to cure. Therefore, the coating films for silver halide photographic light-sensitive materials are difficult to produce liquid scattering by drying air; while the coating films for thermal-developable light-sensitive materials easily produce liquid scattering by drying air. As a result, the coating films for thermal-developable light-sensitive materials have disadvantage of difficulty to obtain good surface condition of coating films, and of easily lowering photographic performance.

**SUMMARY OF THE INVENTION**

The present invention has been worked out taking such situations into account, and the object of the present invention is to provide a method for drying a coating film for a thermal-developable light-sensitive material that can prevent liquid scattering by drying air during drying the coating film for the thermal-developable light-sensitive material; and can achieve good surface condition of the coating film, and good photographic performance.

In order to achieve the above-described object, the present invention is characterized in a method for drying, with drying air in a drying process, a coating film in manufacture of thermal-developable light-sensitive material formed by

coating with a coating liquid that contains an organic silver salt, a reducer for silver ions, a polymer latex, and silver halide particles to a support being conveyed in a coating process, wherein: the drying process comprises: a chilling-zone step for cooling the coating film with cold air; a plane air cushion drying step for a first-stage drying of the coating film in a non-contact state while floating and supporting the support by supplying a hot drying air of a predetermined wind velocity to both sides of the support; a helical air cushion drying step for a second-stage drying of the coating film in a non-contact state while helically winding the support around a circumferential surface of a cylinder and floating and supporting the support by supplying the hot drying air from the circumferential surface of the cylinder to the coating film.

According to the present invention, since second-stage drying, which is full-scale drying, is performed in the helical air cushion drying step, after the coating film has been cured to some extent by the gelation of the coating film in the chilling-zone step, and first-stage drying in the plane air cushion drying step, liquid scattering from the surface of the coating film can be prevented in drying even if the binder has the characteristics of being difficult to cure as in the coating film for the thermal-developable light-sensitive material. Thereby, good surface condition of the coating film and good photographic performance can be achieved.

In the plane air cushion drying step, the wind velocity of drying air is preferably within a range between 20 m/min and 30 m/sec.

For an optimal range of the cold air temperature in the chilling-zone, and the drying air temperature in non-contact drying zone, setting the dry-bulb temperature in the chilling-zone within a range between 5° C. and 50° C. is preferable. It is also preferable to set the dry-bulb temperature in the constant-period of drying in first-stage and second-stage drying within the range between 25° C. and 100° C., and higher than the above-described dry-bulb temperature in the chilling-zone; and to set the wet-bulb temperature within the range between 10° C. and 50° C.

It is preferable that the dry-bulb temperature and the wet-bulb temperature are gradually lowered as the support is conveyed from the entrance side of the plane air cushion drying step toward the exit side of the helical air cushion drying step. Thereby, better surface condition of the coating film and better photographic performance can be achieved.

For an optimal time range from application to dry point, the dry point of the coating film is preferably within 300 seconds after the support is coated with the coating liquid.

For an optimal humidity-controlling time, the humidity-controlling time from the dry point until the support is wound with the winding device is preferably within a range between 10 seconds and 200 seconds.

The coating speed, that is an optimal speed when the support is conveyed from the coating step to the drying step is preferably within a range between 100 m/min and 300 m/min.

**BRIEF DESCRIPTION OF THE DRAWINGS**

The nature of the present invention, as well as other objects and advantages thereof, will be explained in the following with reference to the accompanying drawings, in which like reference characters designate the same or similar parts throughout the figures and wherein:

FIG. 1 is a constitution diagram of a drying process whereto the method for drying a coating film in the manu-

facture of a thermal-developable light-sensitive material according to the present invention, and

FIG. 2 is an explanatory diagram for illustrating equipment for an HAC drying process.

#### DETAILED DESCRIPTION OF THE PREFERRED EMBODIMENTS

A preferred embodiment of the method for drying a coating film for a thermal-developable light-sensitive material according to the present invention will be described in detail below referring to the attached drawings.

FIG. 1 is a constitution diagram of a drying process whereto the method for drying a coating film in the manufacture of a thermal-developable light-sensitive material of the present invention, and the coating step is provided before the drying step.

The coating step 10 is the step for the one-layer application of a coating liquid for a thermal-developable light-sensitive material containing an organic silver salt, a reducer for silver ions, a polymer latex, and silver halide particles on a support 12; or for the simultaneous multi-layer application (three-layer application in FIG. 1) of a coating liquid for a thermal-developable light-sensitive material, a coating liquid to be a protective layer, and the like on a support 12. The coating step 10 mainly comprises a slide-bead applicator 14, and a backup roller 16 for supporting the conveyed support 12. A plurality of coating liquids extruded from the manifold 18 of the slide-bead applicator 14 through a slit 20 onto a slide surface 22 flow down in layers on the slide surface 22, and the support 12 is coated with the coating liquids through a bead formed between the front end of the slide surface and the support 12. Thereby, a coating film is formed on the support 12. The applicator 14 is not limited to a slide-bead applicator, but may be a curtain applicator of other applicators.

The drying step 24 is composed of three steps: a chilling-zone step 26 for cooling the coating film on the support 12 with cold air; a plane air cushion drying step 28 (hereafter referred to as "PAC drying step") for drying the coating film in the non-contact state while floating and supporting the support 12 by supplying hot drying air of a predetermined wind velocity to the both surfaces of the support 12; and a helical air cushion drying step 30 (hereafter referred to as "HAC drying step") for helically winding the support 12 around a tube and drying the coating film in the non-contact state while floating and supporting the support 12 by supplying hot drying air to the coating film from the circumference of the tube.

In the equipment of the chilling-zone step 26, a plurality of pass rollers 34, 35, . . . are arranged along the conveying line of the support 12 in the tunnel-like main body 32 having at both ends thereof an inlet 32A and an outlet 32B for the support 12, and the support 12 is conveyed on the pass roller 34 with the face up. On the upper part of the main body 32 are formed a plurality of supply nozzles 36, 36, . . . for supplying cold air into the main body 32 along the conveying line, and on the lower part of the main body 32 are formed a plurality of exhaust nozzles 38, 38, . . . for discharging the cold air from the main body 32. Thereby, the coating film on the support 12 is cooled by the cold air while being conveyed in the chilling-zone step 26, and the gelation of the coating film is accelerated.

The equipment of the PAC drying step 28 is composed of a plurality of air headers 42, 42, . . . for blowing drying air along the conveying line of the support 12 in the tunnel-like main body 40 having at both ends thereof an inlet 40A and

an outlet 40B for the support 12. The plurality of air headers 42 are arranged in zigzag positions along the conveying line of the support 12. The hot drying air controlled to the wind velocity not to cause the irregularity of and liquid scattering from the coating film surface of the support 12 is blown from the air headers 42 which are arranged in zigzag positions for first-stage drying of the coating film. In this case, the wind velocity that does not cause the irregularity of the coating film surface and liquid scattering after cooling the coating film to accelerate its gelation in the chilling-zone step 26 while exerting the function of the drying air is preferably within a range between 20 m/sec and 30 m/sec. If the wind velocity of the drying air exceeds 30 m/sec, liquid scattering from the coating film surface occurs easily even after the coating film is cooled in the chilling-zone step; and if the wind velocity is lower than 20 m/sec, it is too weak to be the drying air, and drying efficiency is lowered.

The equipment of the HAC drying step 30 is composed of a cylindrical air chamber 44, and a pair of direction-changing units 46 disposed on the both ends of the cylindrical air chamber 44, as shown in the example of the double system in FIG. 2. The cylindrical air chamber 44 is formed cylindrically, and a large number of hole-shaped or slit-shaped air nozzles 48, 48, . . . are formed on the circumferential surface thereof. An air inlet 52 connected to the air pipe 50 is formed on one end surface of the cylindrical air chamber 44, and the hot drying air is supplied from the air source into the cylindrical air chamber 44 and blown out from the air nozzles 48. The support 12 is helically wound around the cylindrical air chamber 44 so that the surface of the coating film becomes involute, and conveyed in the state where a gap (air film) is formed between the coating film and the circumferential surface of the cylindrical air chamber 44 by the pressure of the drying air blown out from the air nozzles 48. Thereby, the coating film is subjected to second-stage drying, which is full-scale drying, by the drying air. The equipment of the HAC drying step 30 is not limited to of the double system, but may be single, or triple or more, depending to the drying conditions.

Each of the direction-changing units 46 is composed of a plurality of cylindrical direction-changing air chambers 54, 54, . . . having semicircular cross sections arranged in parallel, and supports the support 12 so that the direction of the support 12 apart from the helical path of the cylindrical air chamber 44, and the direction of the support 12 entering into the helical path of the cylindrical air chamber 44 become parallel to, but opposite to each other.

Next, the operation of the drying steps composed as described above will be described below.

The support conveyed in the coating step 10 at a coating speed of 100 m/min to 300 m/min is conveyed to the chilling-zone step 26, and the coating film is cooled by the cold air to accelerate the gelation of the coating film. The dry-bulb temperature (D.B.) in the chilling-zone is preferably within a range between 5° C. and 50° C., and the retention time, which is the time required for the support 12 passing through the chilling-zone step 26 is preferably within a range between 10 seconds and 30 seconds. The wind velocity of the cold air in the chilling-zone is preferably within a range between 1 m/sec and 10 m/sec.

The coating film cooled in the chilling-zone step 26 is then conveyed to the PAC drying step 28, the both surfaces of the support 12 are sandwiched by the hot drying air controlled to a predetermined wind velocity, and the coating film is subjected to first-stage drying in a non-contact state. In this first-stage drying, the components of the coating liquid that volatile easily are evaporated.

After previously curing the coating film to some extent by the gelation of the coating film by cooling in the chilling-zone **26** and the evaporation of the components of the coating liquid that volatile easily in the PAC drying step **28**, second-stage drying, which is full-scale drying, of the components of the coating liquid that are difficult to volatile is performed in the HAC drying step **30**. In first-stage drying in the PAC drying step **28** and second-stage drying in the HAC drying step **30**, it is preferable to set the dry-bulb temperature in the constant-period of drying within the range between 25° C. and 100° C., and higher than the dry-bulb temperature in the chilling-zone step **26**; and to set the wet-bulb temperature (W.B.) within the range between 10° C. and 50° C. It is further preferable to set the dry-bulb temperature within the range between 25° C. and 70° C., and higher than the dry-bulb temperature in the chilling-zone step **26**; and to set the wet-bulb temperature within the range between 15° C. and 25° C. It is particularly preferable to set the dry-bulb temperature within the range between 25° C. and 50° C., and higher than the dry-bulb temperature in the chilling-zone step **26**; and to set the wet-bulb temperature within the range between 15° C. and 20° C. In this case, it is preferable to lower the wet-bulb temperature gradually as the support **12** is conveyed from the inlet side of the PAC drying step **28** toward the outlet side of the HAC drying step **30**. This is because the volatile components in the coating liquid decrease as drying of the coating film proceeds, and the temperature of the surface of the coating film elevates unfavorably sharply.

Also, the dry point of the coating film is preferably within 300 seconds after the support **12** is coated with the coating liquid. Therefore, it is recommendable to determine the length of the PAC drying step **28** and the HAC drying step **30** so that the dry point comes in the HAC drying step **30**. Here, the dry point means the point (location) where the equilibrium moisture content is reached; and the equilibrium moisture content means the moisture content when giving and receiving of moisture between the air and the solid (here, the coated support) becomes equilibrium.

The humidity-controlling time from the dry point of the coating film until the support **12** is wound with a winding device (not shown) is preferably within a range between 10 seconds and 200 seconds. This is because constant temperature and constant relative humidity are required to be maintained from the dry point of the coating film until the support **12** is wound by the winding device. The preferable temperature is 20° C. to 30° C., and the preferable relative humidity is 50% to 80%.

As described above, according to the method for drying a coating film for a thermal-developable light-sensitive material of the present invention, since the gelation of the coating film in the chilling-zone step **26** and first-stage drying for evaporating easily volatile components in the PAC drying step **28** are previously performed to cure the coating film to some extent, and then second-stage drying, which is full-scale drying, for evaporating components that are difficult to evaporate is performed in the coating liquid in the HAC drying step **30**, liquid scattering from the surface of the coating film during drying can be prevented, even if the binder has characteristics difficult to cure like the coating film for the thermal-developable light-sensitive material. Therefore, good surface condition of the coating film and good photographic performance can be obtained.

Next, a thermal-developable light-sensitive material preferably used in the present invention will be described in detail below.

Organic silver salts that can be used in the present invention are relatively stable to light; however, when

heated to 80° C. or above in the presence of an exposed photocatalyst (latent image of light-sensitive silver halide and the like) and a reducer, they form silver images. The organic silver salts may be any organic substance containing a source that can reduce silver ions. Such non-light-sensitive organic silver salts are described in Japanese Patent Application Publication No. 10-62899, Paragraph Nos. 0048 and 0049; European Patent Application Publication No. 0803764A1, page 18, line 24 to page 19, line 37; European Patent Application Publication No. 0962812A1; Japanese Patent Application Publication No. 11-349591; Japanese Patent Application Publication No. 2000-7683; and Japanese Patent Application Publication No. 2000-72711. Silver salts of organic acids, and particularly preferable are the silver salts of long-chain aliphatic carboxylic acids (of which the number of carbon atoms is 10 to 30, preferably 15 to 28). Preferable examples of the organic silver salts include silver behenate, silver arachidate, silver stearate, silver oleate, silver laurate, silver capronate, silver myristate, silver palmitate, and the mixture thereof. Of these organic silver salts, the use of an organic silver salt containing 75 mol % or more silver behenate is preferable in the present invention.

The form of the organic silver salts that can be used in the present invention is not specifically limited, and may be needle-like, bar-like, plate-like, and flake-like.

In the present invention, flake-like organic silver salts are preferable. The flake-like organic silver salts are herein defined as follows. When an organic silver salt is observed through an electron microscope, the form of a particle of the organic silver salt is approximately a rectangular parallelepiped, and when the edges of the rectangular parallelepiped are named as a, b, and c from the shortest edge (c may be the same as b), x is calculated from the shorter values a and b as follows:

$$x=b/a$$

Thus, x is calculated for about 200 particles, and when the average is called averaged value x (average), particles that satisfy the relationship of  $x$  (average)  $\geq 1.5$  are defined as flake-shaped. Preferably,  $30 \geq x$  (average)  $\geq 1.5$ , and more preferably,  $20 \geq x$  (average)  $\geq 2.0$ . For reference, a needle-like particle is defined as  $1 \leq x$  (average)  $\leq 1.5$ .

In a flake-like particle, a can be deemed as the thickness of a plate-like particle that has the face having sides band c as the principal face. The average of a is preferably 0.01  $\mu\text{m}$  to 0.23  $\mu\text{m}$ , and more preferably 0.1  $\mu\text{m}$  to 0.20  $\mu\text{m}$ . The average of c/b is preferably 1 or more and 6 or less, more preferably 1.05 or more and 4 or less, further preferably 1.1 or more and 3 or less, and most preferably 1.1 or more and 2 or less.

The distribution of the particle sizes of the organic silver salt is preferably simple distribution. Simple distribution is the distribution when the percentage of the value obtained by dividing the standard deviations of the lengths of the minor axis and the major axis by the minor axis and the major axis, respectively, is 100% or below, more preferably 80% or below, and further preferably 50% or below. The form of the organic silver salt can be measured from the transmission electron microscope image of the dispersion of the organic silver salt. Another method for measuring simple distribution is a method to calculate the standard deviation of the volume-weighted average of the organic silver salt, and the percentage of the value obtained by dividing the standard deviation by the volume-weighted average (coefficient of variation) is preferably 100% or below, more

preferably 80% or below, and further preferably 50% or below. The coefficient of variation can be obtained from the particle size (volume-weighted average diameter) obtained by radiating laser beams to the organic silver salt dispersed in a liquid, and obtaining the autocorrelation function for change in time of the wobble of the scattered light.

Known methods can be applied to the method for manufacturing an organic silver salt used in the present invention and to the method for dispersing it. For example, the above-described Japanese Patent Application Publication No. 10-62899, European Patent Application Publication No. 0803764A1, European Patent Application Publication No. 0962812A1; Japanese Patent Application Publication No. 11-349591; Japanese Patent Application Publication No. 2000-7683; and Japanese Patent Application Publication No. 2000-72711, Japanese Patent Application No. 11-348228, Japanese Patent Application No. 11-348229, Japanese Patent Application No. 11-348230, Japanese Patent Application No. 11-203413, Japanese Patent Application No. 2000-90093, Japanese Patent Application No. 2000-195621, Japanese Patent Application No. 2000-191226, Japanese Patent Application No. 2000-213813, Japanese Patent Application No. 2000-214155, Japanese Patent Application No. 2000-191226, and the like can be referred to.

If a light-sensitive silver salt is allowed to coexist when the organic silver salt is dispersed, fog increases and sensitivity lowers significantly; therefore, it is preferable not to substantially contain light-sensitive silver salts when the organic silver salt is dispersed. In the present invention, the content of light-sensitive silver salts in the aqueous dispersion is 0.1 mol % or less to 1 mole of the organic silver salt in the dispersion, and the light-sensitive silver salts are not intentionally added.

In the present invention, although a light-sensitive material can be manufactured by mixing an aqueous dispersion of an organic silver salt and an aqueous dispersion of a light-sensitive silver salt, and the mixing ratio of the organic silver salt and the light-sensitive silver salt can be selected depending on the purpose, the percentage of the light-sensitive silver salt to the organic silver salt is preferably within a range between 1 mol % and 30 mol %, more preferably within a range between 3 mol % and 20 mol %, and most preferably within a range between 5 mol % and 15 mol %. Mixing two or more aqueous dispersions of organic silver salts and two or more aqueous dispersions of light-sensitive silver salts is a method preferably used for the control of photographic performance.

Although any desired quantity of an organic silver salt can be used in the present invention, the quantity as silver is preferably 0.1 g/m<sup>2</sup> to 5 g/m<sup>2</sup>, and more preferably 1 g/m<sup>2</sup> to 3 g/m<sup>2</sup>.

It is preferable that the thermal-developable light-sensitive material of the present invention contains a reducer for organic silver salts. The reducer for organic silver salts may be any substance (preferably an organic substance) that reduces silver ions to metallic silver. Such reducers are described in Japanese Patent Application Publication No. 11-65021, paragraphs 0043 to 0045; or European Patent Application Publication No. 0803764A1, page 7, line 34 to page 18, line 12.

In the present invention, a hindered phenol reducer and a bisphenol reducer are preferable as the reducer.

In the present invention, the quantity of the reducer is preferably 0.01 g/m<sup>2</sup> to 5.0 g/m<sup>2</sup>, and more preferably 0.1 g/m<sup>2</sup> to 3.0 g/m<sup>2</sup>. For one mole of silver on the surface having an image-forming layer, the content is preferably 5 mol % to 50 mol %, and more preferably 10 mol % to 40 mol %. The reducer is preferably contained in the image-forming layer.

The reducer may be contained in the coating liquid and therefore in the light-sensitive material in any form, such as a dissolved form, an emulsified and dispersed form, and a dispersed fine solid particle form.

One of well-known emulsifying and dispersing methods is a method wherein a reducer is dissolved in oil, such as dibutyl phthalate, tricresyl phosphate, glyceryl triacetate, and diethyl phthalate; or an auxiliary solvent, such as ethyl acetate and cyclohexanone; and then the emulsion is mechanically formed.

Fine solid particle dispersing methods include a method wherein the powder of a reducer is dispersed in a suitable solvent, such as water, using a ball mill, a colloid mill, a vibrating ball mill, a sand mill, a jet mill, a roller mill, or ultrasonic waves to form a solid dispersion. In this time, a protective colloid (for example, polyvinyl alcohol) or a surfactant (for example, an anionic surfactant, such as sodium triisopropylnaphthalenesulfate (mixture of compounds wherein three isopropyl groups are bonded to different substitution sites)) may be used. The aqueous dispersion may contain an antiseptic agent (for example, benzoisothiazolinone sodium salt).

In the thermal-developable light-sensitive material of the present invention, a phenol derivative represented by equation (A) described in Japanese Patent Application No. 11-73951 is preferably used as a developing accelerator.

When the reducer in the present invention has an aromatic hydroxyl group (-OH), especially in the case of the above-described bisphenols, the combined used of a non-reducing compound having groups capable of forming a hydrogen bonds with these groups is preferable. Groups that form hydrogen bonds with hydroxyl or amino groups include phosphoryl, sulfoxide, sulfonyl, carbonyl, amide, ester, urethane, ureido, tertiary amino, and nitrogen-containing aromatic groups. The preferable of these are compounds having a phosphoryl group, a sulfoxide group, an amide group (having no >N-H groups, and blocked as >N-Ra (Ra is a substituent other than H)), a urethane group (having no >N-H groups, and blocked as >N-Ra (Ra is a substituent other than H)), and a ureido group (having no >N-H groups, and blocked as >N-Ra (Ra is a substituent other than H)).

The particularly preferable hydrogen-bondable compound in the present invention is a compound represented by the following general formula (II).

Halogen components in light-sensitive silver halides used in the present invention are not specifically limited, and silver chloride, silver chlorobromide, silver bromide, silver iodobromide, and silver iodochlorobromide can be used. Of these, silver bromide and silver iodobromide are preferable.

The halogen components in a silver halide particle may be evenly distributed, may change stepwise, or may change continuously. Silver halide particles having a core-and-shell structure may also be preferably used. The core-and-shell structure that can be used is preferably a two-layer to five-layer structure, and more preferably a two-layer to four-layer structure. The technique for allowing silver bromide to be locally present on the surfaces of silver chloride or silver chlorobromide particles can also be preferably used.

Methods for forming light-sensitive silver halide are well known to the skilled in the art, and the method described in Research Disclosure, No. 17029, June 1978 and U.S. Pat. No. 3,700,458 can be used. Specifically, a light-sensitive silver halide is formed by adding a silver-providing compound and a halogen-providing compound in a solution of gelatin or other polymers, and then it is mixed with an organic silver salt. Also preferably used are method

described in Japanese Patent Application Publication No. 11-119374, paragraphs 0217 to 0224, and Japanese Patent Application Nos. 11-98708 and 2000-42336.

It is preferably that the particle size of the light sensitive silver halide is small for inhibiting clouding after forming images. Specifically, it is preferably 0.2  $\mu\text{m}$  or smaller, more preferably 0.01  $\mu\text{m}$  or larger and 0.15  $\mu\text{m}$  or smaller, and most preferably 0.02  $\mu\text{m}$  or larger and 0.12  $\mu\text{m}$  or smaller. The term "particle size" used herein is the diameter when the projected area of a silver halide particle (in the case of plate-like particle, the projected area of the major face) is converted to the circular image of the identical area.

The shapes of the silver halide particles include cubic, octahedral, tabular, spherical, rod-like, and potato-like. In the present invention, cubic particles are particularly preferable. Silver halide particles having rounded corners can also be preferably used. The plane index (Miller index) of the outer surfaces of light-sensitive silver halide particles is not specifically limited; however, it is preferable that the percentage of {100} planes, which has a high spectral sensitization efficiency when spectral sensitization dyes are adsorbed, is high. The percentage is preferably 50% or more, more preferably 65% or more, and most preferably 80% or more. The Miller index, the percentage of {100} planes, can be obtained using the method that utilizes the adsorption dependency of {111} planes and {100} planes in the adsorption of the sensitizing dyes, described in T. Tani; J. Imaging Sci., 29, 165 (1985).

In the present invention, silver halide particles having a hexacyano-metal complex existing on the outermost surface thereof are preferable. The hexacyano-metal complexes include  $[\text{Fe}(\text{CN})_6]^{4-}$ ,  $[\text{Fe}(\text{CN})_6]^{3-}$ ,  $[\text{Ru}(\text{CN})_6]^{4-}$ ,  $[\text{Os}(\text{CN})_6]^{4-}$ ,  $[\text{Co}(\text{CN})_6]^{3-}$ ,  $[\text{Rn}(\text{CN})_6]^{3-}$ ,  $[\text{Ir}(\text{CN})_6]^{3-}$ ,  $[\text{Cr}(\text{CN})_6]^{3-}$ , and  $[\text{Re}(\text{CN})_6]^{3-}$ . In the present invention, a hexacyano-iron complex is preferable.

Since hexacyano-metal complexes are present in the form of ions in the aqueous solutions, the counterions are not important; however, the use of alkali-metal ions, such as sodium ions, potassium ions, rubidium ions, cesium ions, and lithium ions; ammonium ions; alkyl ammonium ions (for example, tetramethyl ammonium ions, tetraethyl ammonium ions, tetrapropyl ammonium ions, and tetra (n-butyl) ammonium ions), which are miscible with water and suitable for sedimentation of silver halide emulsions, is preferable.

The hexacyano-metal complexes can be added in the form of water, a mixture with a suitable organic solvent miscible with water (for example, alcohols, ethers, glycols, ketones, esters, amides, and the like), or gelatin.

The quantity of the hexacyano-metal complex added to 1 mole of silver is preferably  $1 \times 10^{-5}$  mole or more and  $1 \times 10^{-2}$  mole or less, and more preferably  $1 \times 10^{-4}$  mole or more and  $1 \times 10^{-3}$  mole or less.

In order to allow the hexacyano-metal complex to be present on the outermost surfaces of silver halide particles, the hexacyano-metal complex is directly added after the addition of the aqueous solution of silver nitrate used for forming particles is completed, and before the charging step up to the chemical sensitizing step for chalcogen sensitization, such as sulfur sensitization, selenium sensitization, and tellurium sensitization, or noble-metal sensitization, such as gold sensitization, is completed, that is, during the water-washing step, the dispersing step, or chemical sensitizing step. In order not to grow the silver halide particles, it is preferable to add the hexacyano-metal complex promptly after the formation of particles, and to add before the completion of the charging step.

The addition of the hexacyano-metal complex may be started after 96% by mass of the total quantity of silver nitrate is added for forming particles, and preferably after 98% by mass is added, and more preferably after 99% by mass is added.

If the hexacyano-metal complex is added after the addition of the aqueous solution of silver nitrate immediately before the completion of the formation of particles, the hexacyano-metal complex can be adsorbed on the outermost surfaces of the silver halide particles, and most of the hexacyano-metal complex reacts with silver ions to form hardly soluble salts. Since the silver salt of hexacyano iron (II) is a harder soluble salt than  $\text{AgI}$ , redissolution by fine particles can be prevented, and the particles of silver halide having a small particle size can be manufactured.

The light-sensitive silver halide particles of the present invention can contain metals or metal complexes of groups 8 to 10 in the periodic table (from group 1 to group 18). The preferable metals in metals or metal complexes of groups 8 to 10 are rhodium, ruthenium, and iridium. These metal complexes may be used alone, or in combination of two or more metals of the same group or of different groups. The content is preferably within a range between  $1 \times 10^{-9}$  mole and  $1 \times 10^{-3}$  mole to 1 mole of the silver. These heavy metals, metal complexes, and methods for the addition thereof are described in Japanese Patent Application Publication No. 7-225449; Japanese Patent Application Publication No. 11-65021, paragraph Nos. 0018 to 0024; and Japanese Patent Application Publication No. 11-119374, paragraph Nos. 0227 to 0240.

Furthermore, metal atoms (for example,  $[\text{Fe}(\text{CN})_6]^{4-}$ ) that can be contained in silver halide particles used in the present invention, and the desalination and chemical sensitization of silver halide emulsions are described in Japanese Patent Application Publication No. 11-84574, paragraph Nos. 0046 to 0050; Japanese Patent Application Publication No. 11-65021, paragraph Nos. 0025 to 0031; and Japanese Patent Application Publication No. 11-119374, paragraph Nos. 0242 to 0250.

Various types of gelatin can be used as the gelatin contained in the light-sensitive silver halide emulsion used in the present invention. In order to maintain the dispersion of the light-sensitive silver halide emulsion in an organic-silver-salt-containing coating liquid, the use of a low-molecular-weight gelatin of a molecular weight of 500 to 60,000 is preferable. Although such a low-molecular-weight gelatin may be used when the particles are formed, or dispersed after desalination treatment, it is preferable to use when the particles are dispersed after desalination treatment.

As a sensitizing dye that can be used in the present invention, a sensitizing dye that can spectrally sensitize silver halide particles in a desired wave-length region when adsorbed on the silver halide particles, and that has a spectral sensitivity commensurate with the spectral properties of the exposing light source can be chosen advantageously. Sensitizing dyes and method for adding are described in Japanese Patent Application Publication No. 11-65021, paragraphs 0103 to 0109; a compound represented by general formula (II) in Japanese Patent Application Publication No. 10-186572; a dye represented by general formula (I) in Japanese Patent Application Publication No. 11-119374, paragraph 0106; U.S. Pat. No. 5,510,236; a dye described in Example 5 of U.S. Pat. No. 3,871,887; a dye disclosed in Japanese Patent Application Publication No. 2-96131 and No. 59-48753; European Patent Application Publication No. 0803764A1, page 19, line 38 to page 20, line 35; Japanese Patent Application Nos. 2000-86865, 2000-102560, and

## 11

2000-205399. These sensitizing dyes may be used alone, or may be used in combination of two or more dyes. In the present invention, the time for adding the sensitizing dye in the silver halide emulsion is preferably after the desalination step up to application, and more preferably after the desalination step and before starting chemical aging.

Although the quantity of the sensitizing dye in the present invention can be any desired quantity to meet the properties of sensitivity or fog, the quantity for 1 mole of the silver halide in the light-sensitive layer is preferably  $10^{-6}$  mole to 1 mole, and more preferably  $10^{-4}$  mole to  $10^{-1}$  mole.

In order to improve the efficiency of spectral sensitization, a strong color sensitizer can be used in the present invention. The strong color sensitizers that can be used in the present invention include compounds described in European Patent Application Publication No. 587,338, U.S. Pat. Nos. 3,877,943 and 4,873,184, and Japanese Patent Application Publication Nos. 5-341432, 11-109547, and 10-111543.

It is preferable that the light-sensitive silver halide particles in the present invention are chemically sensitized by sulfur sensitization, selenium sensitization, or tellurium sensitization. Compounds preferably used in sulfur sensitization, selenium sensitization, and tellurium sensitization are well known to those skilled in the art, and include, for example, a compound described in Japanese Patent Application Publication No. 7-128768. Particularly in the present invention, tellurium sensitization is preferable, and the compounds described in Japanese Patent Application Publication No. 11-65021, paragraph 0030, and the compounds represented by general formulas (II), (III), and (IV) in Japanese Patent Application Publication No. 5-313284 are preferably used.

In the present invention, chemical sensitization can be performed at any time after the formation of particles and before application, and specifically, it can be performed after desalination and (1) before spectral sensitization, (2) at the same time of spectral sensitization, (3) after spectral sensitization, and (4) immediately before application. In particular, it is preferable that chemical sensitization is performed after spectral sensitization.

Although the quantity of sulfur, selenium, and tellurium sensitizers used in the present invention varies depending on silver halide particles used, or the conditions of chemical aging, the quantity for 1 mole of the silver halide is usually  $10^{-8}$  mole to  $10^{-2}$  mole, and preferably  $10^{-7}$  mole to  $10^{-3}$  mole. Although the conditions of chemical sensitization in the present invention are not specifically limited, the pH is preferably 5 to 8, the pAg is preferably 6 to 11, and the temperature is preferably 40° C. to 95° C.

To the silver halide emulsion used in the present invention, a thiosulfonate compound may be added using the method disclosed in European Patent Application Publication No. 293,917.

The light-sensitive silver halide emulsion in the light-sensitive material used in the present invention can be used alone, or two or more light-sensitive silver halide emulsions (for example, of different average particle sizes, different halogen compositions, different crystal habits, or different conditions of chemical sensitization) can be used in combination. The use of a plurality of light-sensitive silver halides of different sensitivities can control the tone. These techniques are disclosed in Japanese Patent Application Publication Nos. 57-119341, 53-106125, 47-3929, 48-55730, 46-5187, 50-73627, and 57-150841. The difference in sensitivity of each emulsion is preferably 0.2 log E or more.

The quantity of the light-sensitive silver halide in terms of the quantity of coating silver for 1 m<sup>2</sup> of the light-sensitive

## 12

material is preferably 0.03 g/m<sup>2</sup> to 0.6 g/m<sup>2</sup>, more preferably 0.07 g/m<sup>2</sup> to 0.4 g/m<sup>2</sup>, and most preferably 0.05 g/m<sup>2</sup> to 0.3 g/m<sup>2</sup>. To 1 mole of the organic silver salt, the quantity of the light-sensitive silver halide is preferably 0.01 mole or more and 0.5 mole or less, and more preferably 0.02 mole or more and 0.3 mole or less.

The methods and conditions for mixing the light-sensitive silver halide and the organic silver salt separately prepared include a method for mixing the prepared silver halide particles and the organic silver salt using a high-speed agitator, a ball mill, a sand mill, a colloid mill, a vibrating mill, or a homogenizer; or a method for mixing the prepared light-sensitive silver halide in some timing during the preparation of the organic silver salt; however, the method is not limited to a specific method as long as the effect of the present invention is obviously obtained. Mixing two or more aqueous dispersions of organic silver salt and two or more aqueous dispersions of light-sensitive silver salt is a preferable method for controlling photographic properties.

Although the time for adding the silver halide in a coating liquid for image forming layers in the present invention is 180 minutes before application to immediately before application, preferably 60 minutes to 10 seconds before application, a method and a condition for mixing are not specifically limited as long as the effect of the present invention is obviously obtained. Specific mixing methods include a method of mixing in a tank wherein the average retention time calculated from the flow rate and the quantity to the coater is controlled to a desired time; or a method to use a static mixer described in N. Harnby, M. F. Edwards, and A. W. Nienow, "Liquid Mixing Techniques", translated by Koji Takahashi, Nikkan Kogyo Shimbun (1989), Chapter 8.

The binder of an organic-silver-salt-containing layer of the present invention may be any polymer, and preferable binders are transparent or translucent, and are generally colorless. They include natural resins, polymers, and copolymers; synthetic resins, polymers, and copolymers; and other media forming films, for example, gelatins, rubbers, polyvinyl alcohols, hydroxyethyl cellulose, cellulose acetate, cellulose acetate butylate, polyvinyl pyrrolidone, casein, starch, polyacrylate, polymethyl methacrylate, polyvinyl chloride, polymethacrylate, styrene-maleic anhydride copolymers, styrene-acrylonitrile copolymers, styrene-butadiene copolymers, polyvinyl acetal (for example, polyvinyl methylal and polyvinyl butylal), polyesters, polyurethane, phenoxy resins, polyvinylidene chloride, polyepoxide, polycarbonate, polyvinyl acetate, polyolefins, cellulose esters, and polyamides. The binders may also be formed by coating from water, organic solvents, or emulsions.

In the present invention, the glass transition temperature of the binder for the layer containing the organic silver salt is preferably 10° C. or above and 80° C. or below (hereinafter also referred to as "high T<sub>g</sub> binder"), more preferably 20° C. to 70° C., and most preferably 23° C. or above and 65° C. or below.

The T<sub>g</sub> herein was calculated using the following equation.

$$1/T_g = \sum (X_i/T_{gi})$$

Here, n monomer components, from i=1 to n, are assumed to copolymerize in the polymer. X<sub>i</sub> is the mass percentage of the i-th monomer ( $\sum X_i = 1$ ), and T<sub>gi</sub> is the glass transition temperature (Kelvin) of the homopolymer of the i-th monomer. Σ is the sum from i=1 to n. The values of the glass transition temperature of homopolymer of each monomer

(Tgi) were taken from J. Brandrup and E. H. Immergut, Polymer Handbook (3rd Edition) (Wiley-Interscience, 1989).

The polymers constituting the binder may be used alone, or used in combination of two or more as required. A polymer having a glass transition temperature of 20° C. or above may be combined with a polymer having a glass transition temperature below 20° C. When two or more polymers having different Tg are blended, it is preferable that the mass average Tg falls in the above-described range.

In the present invention, the performance is improved when the organic-silver-salt-containing layer is formed by coating with a coating liquid containing a solvent whose 30% by mass or more is water, and drying; furthermore, when the binder of the organic-silver-salt-containing layer is soluble or dispersible in a water-based solvent (aqueous solvent); and particularly when the binder is composed of a polymer latex having an equilibrium moisture content at 25° C. and 60% RH of 2% by mass or less. The most preferable aspect is prepared so that the ion conductivity becomes 2.5 mS/cm or below. The methods for preparing such an aspect include purification treatment of the synthesized polymer using a membrane having an isolating function.

The water-based solvent wherein the polymer is soluble or dispersible used herein is water, or the mixture of water and 70% by mass or less water-miscible organic solvent. Water-miscible organic solvents include, for example, alcohols, such as methyl alcohol, ethyl alcohol, and propyl alcohol; cellosolves, such as methyl cellosolve, ethyl cellosolve, and butyl cellosolve; ethyl acetate; and dimethyl formamide.

In the case of a system wherein the polymer is not thermodynamically dissolved, and is present in a so-called dispersed state, the term of a water-based solvent is used here.

The "equilibrium moisture content at 25° C. and 60% RH" is represented by the following equation using the mass of the polymer W1 in a humidity-controlled equilibrium under an atmosphere of 25° C. and 60% RH, and the mass of the polymer W0 in the absolute dry condition at 25° C.

Equilibrium moisture content at 25° C. and 60% RH =  $\{(W1-W0)/W0\} \times 100$  (% by mass).

The definition and the measuring method of moisture content can be referred to, for example, Polymer Engineering Seminar 14, Methods for Testing Polymers (Society of Polymer Science, Japan, Chijin Shokan).

The equilibrium moisture content at 25° C. and 60% RH of the binder polymer of the present invention is preferably 2% by mass or less, more preferably 0.01% by mass or more and 1.5% by mass or less, and most preferably 0.02% by mass or more and 1% by mass or less.

In the present invention a polymer that is dispersible in a water-based solvent is particularly preferable. Examples of dispersed states include a latex wherein fine particles of a hydrophobic polymer insoluble in water are dispersed, and a dispersion of polymer molecules in a molecular state or in a micelle state, both of which are preferable. The average particle diameter of the dispersed particles is preferably within a range between 1 nm and 50,000 nm, and more preferably within a range between 5 nm and 1,000 nm. The particle diameter distribution of the dispersed particles is not specifically limited, and the dispersed particles may have a wide particle diameter distribution or a monodisperse particle diameter distribution.

In the present invention, preferred aspects of polymers dispersible in water-based solvents include hydrophobic polymers, such as acrylic polymers, polyesters, rubber (for

example, SBR resin), polyurethane, polyvinyl chloride, polyvinyl acetate, polyvinylidene chloride, and polyolefins. These polymers may be straight-chain polymers, branched polymers or cross-linked polymers; may be homopolymers wherein a single type of monomers are polymerized; or may be copolymers wherein two or more types of monomers are polymerized. The copolymers may be random copolymers, or may be block copolymers. The molecular weight (number average molecular weight) of these polymers is 5,000 to 1,000,000, preferably 10,000 to 200,000. If the molecular weight is too low, the mechanical strength of the emulsion layer is insufficient; and if the molecular weight is too high, the film forming capability becomes poor.

Specific examples of preferable latexes are listed below. The list shows material monomers, the unit of values in parentheses is % by mass, and molecular weights are number average molecular weights. In the case of poly-functional monomers, since the concept of molecular weight cannot be applied because they form cross-linked structures, they are described as "cross-linkable", and the description of molecular weights is omitted. Tg denotes glass transition temperature. p0 P-1; -MMA (70)-EA (27)-MAA (3)-latex (molecular weight: 37,000) p0 P-2; -MMA (70)-2EHA (20)-St (5)-AA (5)-latex (molecular weight: 40,000) p0 P-3; -St (50)-Bu (47)-MAA (3)-latex (cross-linkable) p0 P-4; -St (68)-Bu (29)-AA (3)-latex (cross-linkable) p0 P-5; -St (71)-Bu (26)-AA (3)-latex (cross-linkable, Tg 24° C.) p0 P-6; -St (70)-Bu (27)-IA (3)-latex (cross-linkable) p0 P-7; -St (75)-Bu (24)-AA (1)-latex (cross-linkable) p0 P-8; -St (60)-Bu (35)-DVB (3)-MAA (2)-latex (cross-linkable) p0 P-9; -St (70)-Bu (25)-DVB (2)-AA (3)-latex (cross-linkable) p0 P-10; -VC (50)-MMA (20)-BA (20)-AN (5)-AA (3)-latex (molecular weight: 80,000) p0 P-11; -VDC (85)-MMA (5)-EA (5)-MAA (5)-latex (molecular weight: 67,000) p0 P-12; -Et (90)-MMA (10)-latex (molecular weight: 12,000) p0 P-13; -St (70)-2EHA (27)-AA (3)-latex (molecular weight: 130,000) p0 P-14; -MMA (63)-EA (35)-AA (2)-latex (molecular weight: 33,000) p0 P-15; -St (70.5)-Bu (26.5)-AA (3)-latex (cross-linkable, Tg 23° C.) p0 P-16; -St (69.5)-Bu (27.5)-AA (3)-latex (cross-linkable, Tg 20.5° C.)

Abbreviations in the above-described structures denote the following monomers: MMA: methyl methacrylate, EA: ethyl acrylate, MAA: methacrylic acid, 2EHA: 2-ethylhexyl acrylate, St: styrene, Bu: butadiene, AA: acrylic acid, DVB: divinyl benzene, VC: vinyl chloride, AN: acrylonitrile, VDC: vinylidene chloride, Et: ethylene, IA: itaconic acid.

The above-described polymer latexes are also sold in the market, and the following polymers are commercially available. Examples of acrylic polymers include Cevian A-4635, 4718, and 4601 (Daicel Chemical Industries) and Nipol Lx 811, 814, 821, 820, and 857 (ZEON Corporation); examples of polyesters include FINETEX ES 650, 611, 675, and 850 (Dainippon Ink and Chemicals, Inc.) and WD-size and WMS (Eastman Chemical); examples of polyurethane include HYDRAN AP 10, 20, 30, and 40 (Dainippon Ink and Chemicals, Inc.); examples of rubbers include LACSTAR 7301K, 3307B, 4700H, and 7132C (Dainippon Ink and Chemicals, Inc.) and Nipol Lx 416, 410, 438C, and 2507 (ZEON Corporation); examples of polyvinyl chloride include G351 and G576 (ZEON Corporation); examples of polyvinylidene chloride include L502 and L513 (Asahi Kasei); and examples of polyolefins include Chemipearl S120 and SA100 (Mitsui Chemicals).

These polymer latexes may be used alone, or may be used in combination of two or more as required.

The polymer latex preferably used in the present invention is latex of a styrene-butadiene copolymer. The mass

ratio of styrene monomer units to butadiene monomer units in the styrene-butadiene copolymer is preferably 40:60 to 95:5. The proportion of styrene monomer units and butadiene monomer units in the copolymer is preferably 60% by mass to 99% by mass. The preferable molecular weight range is the same as described above.

Latexes of styrene-butadiene copolymers preferably used in the present invention include the above-described P-3 to P-8, P-14, P-15, commercially available LACSTAR-3307B, 7132C, and Nipol Lx 416.

In the organic-silver-salt-containing layer of the light-sensitive material of the present invention, hydrophilic polymers, such as gelatin, polyvinyl alcohol, methylcellulose, hydroxypropyl cellulose, and carboxymethyl cellulose may be added as required. The content of these hydrophilic polymers in the total quantity of binders in the organic-silver-salt-containing layer is preferably 30% by mass or less, and more preferably 20% by mass or less.

The organic-silver-salt-containing layer (image forming layer) of the present invention is preferably formed from polymer latex. The mass ratio of the total quantity of the binder to the organic silver salt in the organic-silver-salt-containing layer is within a range between 1/10 and 10/1, preferably 1/5 and 4/1.

Such an organic-silver-salt-containing layer is normally a light-sensitive layer (emulsion layer) containing light-sensitive silver halide, which is a light-sensitive silver salt, and in this case, the mass ratio of total binders to the silver halide is within a range between 400 and 5, preferably 200 to 10.

The total quantity of the binder in the image-forming layer of the present invention is within a range between 0.2 g/m<sup>2</sup> and 30 g/m<sup>2</sup>, preferably between 1 g/m<sup>2</sup> and 15 g/m<sup>2</sup>. In the image-forming layer of the present invention, a cross-linking agent for cross-linking, and a surfactant for improving coating properties may be added.

In the present invention, the solvent (here, a solvent and a dispersant are collectively referred to as solvent for simplification) in the coating liquid for the organic-silver-salt-containing layer of the light-sensitive layer in the present invention is preferably a water-based solvent containing 30% by mass or more water. The components other than water may be any optional water-miscible organic solvents, such as methyl alcohol, ethyl alcohol, isopropyl alcohol, methyl cellosolve, ethyl cellosolve, dimethyl formamide and ethyl acetate. The water content in the solvent of the coating liquid is preferably 50% by mass or more, and more preferably 70% by mass or more. The preferable examples of solvent compositions are water, water/methyl alcohol=90/10, water/methyl alcohol=70/30, water/methyl alcohol/dimethyl formamide=80/15/5, water/methyl alcohol/ethyl cellosolve=85/10/5, and water/methyl alcohol/isopropyl alcohol=85/10/5 (unit: % by mass).

The anti-fog agent, stabilizer, and precursor for the stabilizer that can be used in the present invention include compounds described in Japanese Patent Application Publication No. 10-62899, paragraph 0070, European Patent Application Publication No. 0803764A1, page 20, line 57 to page 21, line 7, and Japanese Patent Application Publication Nos. 9-281637 and 9-329864. The anti-fog agents preferably used in the present invention are organic halogen compounds, and are disclosed in Japanese Patent Application Publication No. 11-65021, paragraphs 0111 to 0112. The organic halogen compounds represented by formula (P) of Japanese Patent Application No. 11-87297, the organic polyhalogen compound represented by general formula (II) of Japanese Patent Application Publication No. 10-339934,

and the organic polyhalogen compounds described in Japanese Patent Application No. 11-205330 are particularly preferable.

The organic polyhalogen compounds preferably used in the present invention will specifically be described below. The preferable polyhalogen compounds are compounds represented by the following general formula (III).

General Formula (III)



In general formula (III), Q represents an alkyl group, aryl group, or heterocyclic group; Y represents a divalent coupling group; n represents 0 or 1; Z1 and Z2 represent halogen atoms; and X represents a hydrogen atom or an electron-attracting group. In general formula (III), Q is preferably a phenyl group substituted by an electron-attracting group whose Hammett substituent constant  $\sigma$  is positive. The Hammett substituent constant is described in Journal of Medicinal Chemistry, 1973, Vol. 16, No. 11, pp. 1207-1216. Such electron-attracting groups include, for example, halogen atoms (fluorine atom ( $\sigma$  value: 0.06), chlorine atom ( $\sigma$  value: 0.23), bromine atom ( $\sigma$  value: 0.23), iodine atom ( $\sigma$  value: 0.18)), trihalomethyl groups (tribromomethyl ( $\sigma$  value: 0.29), trichloromethyl ( $\sigma$  value: 0.33), trifluoromethyl ( $\sigma$  value: 0.54)), cyano group ( $\sigma$  value: 0.66), nitro group ( $\sigma$  value: 0.78), aliphatic aryl or heterocyclic sulfonyl groups (for example, methane sulfonyl ( $\sigma$  value: 0.72)), aliphatic aryl or heterocyclic acyl groups (for example, acetyl ( $\sigma$  value: 0.50), benzoyl ( $\sigma$  value: 0.43)), alkynyl groups (for example,  $C\equiv CH$  ( $\sigma$  value: 0.23)), aliphatic aryl or heterocyclic oxycarbonyl groups (for example, methoxy carbonyl ( $\sigma$  value: 0.45), phenoxy carbonyl ( $\sigma$  value: 0.44)), carbamoyl group ( $\sigma$  value: 0.36), sulfamoyl groups ( $\sigma$  value: 0.57), sulfoxide groups, heterocyclic groups, and phosphoryl groups. The  $\sigma$  value is preferably within a range between 0.2 and 2.0, more preferably within a range between 0.4 and 1.0. Particularly preferable electron-attracting groups are carbamoyl, alkoxy carbonyl, alkylsulfonyl, and alkyl phosphoryl groups, of which the most preferable is the carbamoyl group.

X represents preferably an electron-attracting group, more preferably a halogen atom, an aliphatic aryl or heterocyclic sulfonyl group, an aliphatic aryl or heterocyclic acyl group, an aliphatic aryl or heterocyclic oxycarbonyl group, a carbamoyl group, and a sulfamoyl group, and particularly preferably a halogen atom. Among halogen atoms, a chlorine atom, bromine atom, and iodine atom are preferable; a chlorine atom and bromine atom are more preferable; and a bromine atom is most preferable.

Y represents preferably  $-C(=O)-$ ,  $-SO_2-$ , or  $-SO_2-$ , more preferably  $-C(=O)-$  or  $-SO_2-$ , and most preferably  $-SO_2-$ . n represents 0 or 1, preferably 1.

In the present invention, the methods for containing an anti-fog agent in the light-sensitive material include the method described in the above-described method for containing the reducer, and the addition of fine solid particles is also preferable for the organic polyhalogen compound.

Other anti-fog agents include the mercury (II) salt in Japanese Patent Application Publication No. 11-65021, paragraph 0113, benzoates in Japanese Patent Application Publication No. 11-65021, paragraph 0114, salicylic acid derivatives in Japanese Patent Application Publication No. 2000-206642, formalin scavenger compounds represented by formula (S) in Japanese Patent Application Publication No. 2000-221634, triazine compounds according to claim 9 of Japanese Patent Application Publication No. 11-352624,

the compounds represented by general formula (III) of Japanese Patent Application Publication No. 6-11791, and 4-hydroxy-6-methyl-1,3,3a,7-tetrazaindene.

The thermal-developable light-sensitive material of the present invention may contain an azonium salt for the purpose of preventing fog. The azonium salts include the compounds represented by general formula (XI) described in Japanese Patent Application Publication No. 59-193447, the compound described in Japanese Patent publication No. 55-12581, and the compounds represented by general formula (II) described in Japanese Patent Application Publication No. 60-153039. Although the azonium salt can be added to any positions in the light-sensitive material, addition to the layer on the surface having the light-sensitive layer is preferable, and addition to the organic-silver-salt-containing layer is more preferable. Although the azonium salt can be added in any steps for the preparation of the coating liquid, and when it is added to the organic-silver-salt-containing layer, it can be added in any steps from the time for the preparation of the organic silver salt to the preparation of the coating liquid, and preferably the time after the preparation of the organic silver salt to immediately before coating. The azonium salt may be added in any forms, such as powder, a solution, and a dispersion of fine particles. It may also be added as a solution whereto other additives, such as a sensitizing dye, a reducer, and toning agent, are added. In the present invention, although the quantity of the azonium salt to be added may be optional, it is preferably  $1 \times 10^{-6}$  mole or more and 2 moles or less, and more preferably  $1 \times 10^{-3}$  mole or more and 0.5 moles or less to 1 mole of silver.

In the present invention, a mercapto compound, a disulfide compound, and a thion compound may be contained for inhibiting, accelerating, or controlling development; for improving the efficiency of spectral sensitization; and for improving storage stability before and after development. The specific examples are described in Japanese Patent Application Publication No. 10-62899, paragraphs 0067 to 0069; the compounds represented by general formula (I) of Japanese Patent Application Publication No. 10-186572, and paragraphs 0033 to 0052; European Patent Application Publication No. 0803764A1, page 20, lines 36 to 56; and Japanese Patent Application No. 11-273670. Above all, a mercapto-substituted heterocyclic aromatic compound is preferable.

In the thermal-developable light-sensitive material of the present invention, the addition of a toning agent is preferable. Toning agents are described in Japanese Patent Application Publication No. 10-62899, paragraph Nos. 0054 and 0055; European Patent Application Publication No. 0803764A1, page 21, lines 23 to 48; Japanese Patent Application Publication No. 2000-356317; and Japanese Patent Application No. 2000-187298. Particularly preferable are phthaladinones (phthaladinone, phthaladinone derivatives, or metal salts; for example, 4-(1-naphthyl) phthaladinone, 6-chlorophthaladinone, 5,7-dimethoxyphthaladinone, and 2,3-dihydro-1,4-phthaladinedione); the combination of phthaladinones and phthalates (for example, phthalic acid, 4-methyl phthalic acid, 4-nitro phthalic acid, diammonium phthalate, sodium phthalate, potassium phthalate, and tetrachloro phthalic anhydride); phthaladines (phthaladine, phthaladine derivatives, or metal salts; for example, 4-(1-naphthyl) phthaladine, 6-isopropyl phthaladine, 6-t-butyl phthaladine, 6-chloro phthaladine, 5,7-dimethoxy phthaladine, and 2,3-dihydro phthaladine); and the combination of phthaladines and phthalates. Of these, the combination of phthaladines and phthalates is most preferable.

Plasticizers and lubricants that can be used in the light-sensitive layers of the present invention are described in

Japanese Patent Application Publication No. 11-65021, paragraph 0117; the super-high contrast agents for forming super-high contrast images, and the method of addition and quantity thereof are described in Japanese Patent Application Publication No. 11-65021, paragraph 0118; Japanese Patent Application Publication No. 11-223898, paragraphs 0136 to 0193; Japanese Patent Application No. 11-87297, compounds of formulas (H), (1) to (3), (A), and (B); Japanese Patent Application No. 11-91652, compounds of general formulas (III) to (V) (specific compounds: compounds 21 to 24); and high-contrast promoters are described in Japanese Patent Application Publication No. 11-65021, paragraph 0102, and Japanese Patent Application Publication No. 11-223898, paragraphs 0194 and 0195.

In order to use formic acid or a formate as a strong fogging substance, it is preferably contained in the side having an image-forming layer that contains the light-sensitive silver halide in a quantity of 5 mmol or less for 1 mole of silver, more preferably 1 mmol or less.

When an ultra-high contrast agent is used in the thermal-developable light-sensitive material of the present invention, it is preferable to use in combination with an acid or the salt thereof formed by hydrating diphosphorus pentoxide. The acids or the salts thereof formed by hydrating diphosphorus pentoxide include metaphosphoric acid (metaphosphates), pyrophosphoric acid (pyrophosphates), orthophosphoric acid (orthophosphates), triphosphoric acid (triphosphates), tetraphosphoric acid (tetraphosphates), and hexametaphosphoric acid (hexametaphosphates). Particularly preferable acids or the salts thereof formed by hydrating diphosphorus pentoxide are orthophosphoric acid (orthophosphates), and hexametaphosphoric acid (hexametaphosphates). Specific salts include sodium orthophosphate, dihydrogen sodium orthophosphate, sodium hexametaphosphate, and ammonium hexametaphosphate.

Although the quantity (coating quantity for 1 m<sup>2</sup> of the light-sensitive material) of acids or the salts thereof formed by hydrating diphosphorus pentoxide may be as desired depending on the performance, such as sensitivity and fog, it is preferably 0.1 mg/m<sup>2</sup> to 500 mg/m<sup>2</sup>, and more preferably 0.5 mg/m<sup>2</sup> to 100 mg/m<sup>2</sup>.

The thermal-developable light-sensitive material of the present invention may have a surface-protecting layer for the purpose of preventing the adherence of the image-forming layer. The surface-protecting layer may be of a single layer, or may be of multiple layers. The surface-protecting layer is described in Japanese Patent Application Publication No. 11-65021, paragraphs 0119 to 0120, and Japanese Patent Application No. 2000-171936.

Although gelatin is preferably used for the binder of the surface-protecting layer of the present invention, it is also preferable to use or to combine polyvinyl alcohol (PVA). Gelatin that can be used include inert gelatin (for example, Nitta Gelatin 750) and phthalated gelatin (for example, Nitta Gelatin 801). PVA that can be used is described in Japanese Patent Application Publication No. 2000-171936, paragraphs 0009 to 0020, and fully saponified PVA-105, partially saponified PVA-205, PVA-335, and modified polyvinyl alcohol MP-203 (KURARAY) are preferably used. The quantity of polyvinyl alcohol coating as the protecting layer (per layer) (per 1 m<sup>2</sup> of the support) is preferably 0.3 g/m<sup>2</sup> to 4.0 g/m<sup>2</sup>, and more preferably 0.3 g/m<sup>2</sup> to 2.0 g/m<sup>2</sup>.

Particularly, when the thermal-developable light-sensitive material of the present invention is used for printing, wherein change in dimensions raises problems, the use of

polymer latex in the surface-protecting layer or the backing layer is preferable. Such polymer latexes are described in Taira Okuda and Hiroshi Inagaki, "Synthetic Resin Emulsion", Kobunshi Kankoukai (1978); Takaaki Sugimura, Yasuo Kataoka, Soichi Suzuki, and Keiji Kasahara, "Application of Polymer Latex", Kobunshi Kankoukai (1993); and Soichi Muroi, "Chemistry of Polymer Latex", Kobunshi Kankoukai (1970). Specifically, the polymer latexes include a latex of methyl methacrylate (33.5% by mass)/ethyl acrylate (50% by mass)/methacrylic acid (16.5% by mass) copolymer; a latex of methyl methacrylate (47.5% by mass)/butadiene (47.5% by mass)/itaconic acid (5% by mass) copolymer; a latex of ethyl acrylate/methacrylic acid copolymer; a latex of methyl methacrylate (58.9% by mass)/2-ethylhexyl acrylate (25.4% by mass)/styrene (8.6% by mass)/2-hydroxyethyl methacrylate (5.1% by mass)/acrylic acid (2.0% by mass) copolymer; and a latex of methyl methacrylate (64.0% by mass)/styrene (9.0% by mass)/butyl acrylate (20.0% by mass)/2-hydroxyethyl methacrylate (5.0% by mass)/acrylic acid (2.0% by mass) copolymer. Furthermore, the combination of polymer latexes described in Japanese Patent Application No. 11-6872, the technique described in Japanese Patent Application No. 11-143058, paragraphs 0021 to 0025; the technique described in Japanese Patent Application No. 11-6872, paragraphs 0027 to 0028; and the technique described in Japanese Patent Application No. 10-199626, paragraphs 0023 to 0041 can be applied to binders for surface-protecting layer. The content of the polymer latex for surface-protecting layer is preferably 10% by mass to 90% by mass of the total binder, more preferably 20% by mass to 80% by mass.

The quantity of the total binders (including water-soluble polymers and latex polymers) of the surface-protecting layer (per layer) (per 1 m<sup>2</sup> of the support) is preferably 0.3 g/m<sup>2</sup> to 5.0 g/m<sup>2</sup>, and more preferably 0.3 g/m<sup>2</sup> to 2.0 g/m<sup>2</sup>.

The temperature in the preparation of the coating liquid for the image-forming layer in the present invention is 30° C. or above and 65° C. or below, preferably 35° C. or above and below 60° C., and more preferably 35° C. or above and 55° C. or below. It is also preferable that the temperature of the coating liquid for the image-forming layer immediately after the addition of polymer latex is maintained at 30° C. or above and 65° C. or below.

The image-forming layer of the present invention is composed of one or more layer on the support. When it is composed of one layer, the layer comprises an organic silver salt, light-sensitive silver halide, a reducer, and a binder, and as required, contains additional materials, such as a toning agent, covering additives and other auxiliary agents. When it is composed of two or more layers, the first image-forming layer (normally the layer contacting the support) must contain an organic silver salt and light-sensitive silver halide, and the second image-forming layer or both layers must contain other several components. The constitution of a multicolor light-sensitive thermal-developable photographic material may contain the combination of these two layers for each color, and all the components may be contained in a single layer, as described in U.S. Pat. No. 4,708,928. In the case of a multi-dye multicolor light-sensitive thermal-developable photographic material, each emulsion layer is separated from each other and maintained by using a functional or non-functional barrier layer between each light-sensitive layer, as described in U.S. Pat. No. 4,460,681.

Various dyes or pigments (for example, C. I. Pigment Blue 60, C. I. Pigment Blue 64, and C. I. Pigment Blue 15:6) can be used in the light-sensitive layer of the present

invention from the point of view of improving color tone, preventing the occurrence of interference fringes in exposing a laser beam, and preventing irradiation. These are described in WO 98/36322, and Japanese Patent Application Publication Nos. 10-268465 and 11-338098.

In the thermal-developable light-sensitive material of the present invention, an anti-halation layer can be provided on the side of light-sensitive layer remote from the light source.

A thermal-developable light-sensitive material has generally non-light-sensitive layers in addition to a light-sensitive layer. Non-light-sensitive layers can be classified according to the location thereof into (1) a protecting layer provided on the light-sensitive layer (remote side from the support), (2) an intermediate layer provided between a plurality of light-sensitive layers or between the light-sensitive layer and the protecting layer, (3) a primer layer provided between the light-sensitive layer and the support, and (4) a backing layer provided on the side opposite to the light-sensitive layer. A filter layer is provided on the light-sensitive layer as the layer (1) or (2). The anti-halation layer is provided on the light-sensitive layer as the layer (3) or (4).

Anti-halation layers are described in, for example, Japanese Patent Application Publication No. 11-65021, paragraphs 0123 and 0124; Japanese Patent Application Publication Nos. 11-223898, 9-230531, 10-36695, 10-104779, 11-231457, 11-352625, and 11-352626.

The anti-halation layer contains an anti-halation dye having absorption in the exposure wavelength. When the exposure wavelength is in the infrared region, an infrared absorbing dye can be used, and in this case, the dye that has no absorption in the visible region is preferable.

If halation is prevented using a dye having absorption in the visible region, it is preferable that the color of the dye does not substantially remain after forming images, a means to vanish the color with the heat of thermal development is used, and in particular, a thermally achromatizing dye and a base precursor are added to a non-light-sensitive layer to function as an anti-halation layer. These techniques are described in Japanese Patent Application Publication No. 11-231457.

The quantity of the achromatizing dye is determined according to the use of the dye. In general, it is used in a quantity that the optical density (absorbance) measured by the objective wavelength exceeds 0.1. The optical density is preferably 0.2 to 2. The quantity of the dye for obtaining such an optical density is generally approximately 0.001 g/m<sup>2</sup> to 1 g/m<sup>2</sup>.

When the dye is achromatized, the optical density after thermal development can be lowered to 0.1 or less. Two or more achromatizing dyes may be used in combination in a thermally achromatizing recording material or a thermal-developable light-sensitive material. Similarly, two or more base precursors may be used in combination.

In thermal achromatizing using such achromatizing dyes and base precursors, the combination use of a substance that lowers the melting point by 3 degrees or more by mixing with a base precursor such as described in Japanese Patent Application Publication No. 11-352626 (for example, diphenylsulfone and 4-chloroprene (phenyl) sulfide) is preferable from the point of view of thermal achromatizing.

In the present invention, for the purpose of improving change by aging of the silver color tone and the images, a colorant having an absorption maximum at 300 nm to 450 nm can be added. Such a colorant is described, for example, in Japanese Patent Application Publication Nos. 62-210458, 63-104046, 63-103235, 63-208846, 63-306436, 63-314535, 01-61745, and Japanese Patent Application No. 11-276751.

Such a colorant is normally added within a range between 0.1 mg/m<sup>2</sup> and 1 mg/m<sup>2</sup>, and the layer for the addition of the colorant is preferably the back layer provided opposite to the light-sensitive layer.

The thermal-developable light-sensitive material in the present invention is preferably a one-sided light-sensitive material having at least one light-sensitive layer containing a silver halide emulsion on one side of the support, and having a backing layer on the other side.

In the present invention, it is preferable to add a mat agent for improving conveying properties, and the mat agent is described in Japanese Patent Application Publication No. 11-65021, paragraphs 0126 to 0127. The quantity of the mat agent coating for 1 m<sup>2</sup> of the light-sensitive material is preferably 1 mg/m<sup>2</sup> to 400 mg/m<sup>2</sup>, and more preferably 5 mg/m<sup>2</sup> to 300 mg/m<sup>2</sup>.

Although any mat degree of the emulsion surface is optional unless stardust defects occur, the Peck flatness is preferably 30 seconds or more and 2,000 seconds or less, and more preferably 40 seconds or more and 1,500 seconds or less. The Peck flatness can be obtained in accordance with Japanese Industrial Standards (JIGS) P8119, "Method for Testing Flatness of Paper and Cardboard Using Peck Tester", and TAPIR Standard Method T479.

In the present invention, the Peck flatness for a mat degree of the backing layer is preferably 1,200 seconds or less and 10 seconds or more, more preferably 800 seconds or less and 20 seconds or more, and most preferably 500 seconds or less and 40 seconds or more.

In the present invention, the matting agent is preferably contained in the outermost surface layer of the light-sensitive layer or a layer that functions as the outermost surface layer, a layer close to the outer surface, or a layer that functions as the protecting layer.

The backing layer that can be applied to the present invention is described in Japanese Patent Application Publication No. 11-65021, paragraphs 0128 to 0130.

The pH of the film surface of the thermal-developable light-sensitive material before thermal development in the present invention is preferably 7.0 or lower, and more preferably 6.6 or lower. Although the lower limit thereof is not specifically limited, it is about 3. The most preferable pH range is between 4 and 6.2. The control of the pH of the film surface using an organic acid such as phthalic acid derivatives, a non-volatile acid such as sulfuric acid, or a volatile base such as ammonia is preferable from the point of view of lowering the pH of the film surface. In particular, since ammonia is easily evaporated and can be removed before the coating step or thermal development, it is preferable for achieving a low pH of the film surface.

The combined use of a non-volatile base, such as sodium hydroxide, potassium hydroxide, and lithium hydroxide, with ammonia is also preferable. A method for measuring the pH of the film surface is described in Japanese Patent Application No. 11-87297, paragraph 0123.

In the layers of the present invention, such as light-sensitive layer, the protecting layer, and the backing layer, a hardener can be used. Examples of hardeners include methods described in T. H. James, "The Theory of the Photographic Process, Fourth Edition", Macmillan Publishing Co. Inc, (1977), pages 77 to 87; and chrome alum, 2,4-dichloro-6-hydroxy-s-triazine sodium salt, N,N-ethylene bis(vinylsulfone acetamide), and N,N-propylene bis(vinylsulfone acetamide); as well as multivalent metal ions described in page 78 of the same reference book; polyisocyanates described in U.S. Pat. No. 4,281,060 and Japanese Patent Application Publication No. 6-208193; epoxy com-

pounds described in U.S. Pat. No. 4,791,042; and vinylsulfone-based compounds described in Japanese Patent Application Publication No. 62-89048 are preferably used.

The hardener is added in the form of a solution, and the time for adding the solution to the coating liquid for the protecting layer is 180 minutes before to immediately before coating, preferably 60 minutes to 10 seconds before coating. The methods and conditions for mixing are not specifically limited as long as the effect of the present invention is sufficiently achieved. Specific methods for mixing include a method of mixing in a tank wherein the average retention time calculated from the flow rate and the quantity to the coater is controlled to a desired time; or a method to use a static mixer described in N. Harnby, M. F. Edwards, and A. W. Nienow, "Liquid Mixing Techniques", translated by Koji Takahashi, Nikkan Kogyo Shimbun (1989), Chapter 8.

The surfactants, the solvent, the support, the anti-static or conductive layer, and the method for obtaining color images that can be used in the present invention are disclosed in Japanese Patent Application Publication No. 11-65021, paragraph 0132, 0133, 0134, 0135, and 0136, respectively; and the lubricants are described in Japanese Patent Application Publication No. 11-84573, paragraphs 0061 to 0064, and Japanese Patent Application No. 11-106881, paragraphs 0049 to 0062.

For a transparent support, polyester, especially polyethylene terephthalate undergone heat treatment within a temperature range between 130° C. and 185° C. is preferably used for relieving internal strain remaining in the film during biaxial drawing, and eliminating thermal shrinkage strain occurring during thermal development. In the case of a thermal-developable light-sensitive material, the transparent support may be colored with a blue dye (for example, dye-1 described in Japanese Patent Application Publication No. 8-240877), or may be not colored. It is preferable that the primer techniques of water-soluble polyester described in Japanese Patent Application Publication No. 11-84574, styrene-butadiene copolymer described in Japanese Patent Application Publication No. 10-186565, and vinylidene chloride copolymers described in Japanese Patent Application Publication No. 2000-39684 and Japanese Patent Application No. 11-106881, paragraphs 0063 to 0080 are applied to the support. To the antistatic layers or the primers, the techniques described in Japanese Patent Application Publication Nos. 56-143430, 56-143431, 58-62646, 56-120519, and 11-84573, paragraphs 0040 to 0051, U.S. Pat. No. 5,575,957, and Japanese Patent Application Publication No. 11-223898, paragraphs 0078 to 0084 can be applied.

The thermal-developable light-sensitive material is preferably of a monosheet type (a type that can form images on a thermal-developable light-sensitive material not using other sheets as in image-receiving materials).

To the thermal-developable light-sensitive material, an anti-oxidant, a stabilizer, a plasticizer, a ultraviolet absorber, or coating additives may further be added. The various additives are added to either the light-sensitive layer or a non-light-sensitive layer. These are described in WO 98/36322, EP 803764A1, Japanese Patent Application Publication Nos. 10-186567 and 10-18568.

The thermal-developable light-sensitive material in the present invention can be applied using any methods. Specifically, various coating operations can be used, including extrusion coating, slide coating, curtain coating, dip coating, knife coating, flow coating, and extrusion coating using a hopper of a type described in U.S. Pat. No. 2,681,294. Extrusion coating described in Stephen F. Kistler, Peter M. Schweizer, "Liquid Film Coating", (Chapman & Hall,

1997), pages 399 to 536, or slide coating are preferably used, and slide coating is most preferably used. An example of a form of slide coaters used for slide coating is shown in FIG. 11b.1 in page 427 of the above-described reference. If desired, two or more layers can be applied simultaneously using the methods described in pages 399 to 536 of the above-described reference, U.S. Pat. No. 2,761,791, and British Patent No. 837,095.

The organic-silver-salt-containing coating liquid in the present invention is preferably a so-called thixotropic fluid. This technique is described in Japanese Patent Application Publication No. 11-52509. The viscosity at a shear rate of 0.1 s<sup>-1</sup> of the coating liquid is preferably 400 mPa·s or more and 100,000 mPa·s or less, and more preferably 500 mPa·s or more and 200,000 mPa·s or less. The viscosity at a shear rate of 1000 s<sup>-1</sup> is preferably 1 mPa·s or more and 200 mPa·s or less, and more preferably 5 mPa·s or more and 80 mPa·s or less.

Techniques that can be used in the thermal-developable light-sensitive material of the present invention are also described in EP 803764A1, EP 883022A1, WO 98/36322, Japanese Patent Application Publication Nos. 56-62648, 58-62644, 9-43766, 9-281637, 9-297367, 9-304869, 9-311405, 9-329865, 10-10669, 10-62899, 10-69023, 10-186568, 10-90823, 10-171063, 10-186565, 10-186567, 10-186569, 10-186570, 10-186571, 10-186572, 10-197974, 10-197982, 10-197983, 10-197985, 10-197986, 10-197987, 10-207001, 10-207004, 10-221807, 10-282601, 10-288823, 10-288824, 10-307365, 10-312038, 10-339934, 11-7100, 11-15105, 11-24200, 11-24201, 11-30832, 11-84574, 11-65021, 11-109547, 11-125880, 11-129629, 11-133536, 11-133537, 11-133538, 11-133539, 11-133542, 11-133543, 11-223898, 11-352627, 11-305377, 11-305378, 11-305384, 11-305380, 11-316435, 11-327076, 11-338096, 11-338098, 11-338099, 11-343420, Japanese Patent Application Nos. 2000-187298, 2000-10229, 2000-47345, 2000-206642, 2000-98530, 2000-98531, 2000-112059, 2000-112060, 2000-112104, 2000-112064, 2000-171936, and 11-282190.

The thermal-developable light-sensitive material of the present invention may be developed using any methods, and normally, it is developed by heating the thermal-developable light-sensitive material exposed image-wise. The developing temperature is preferably 80° C. to 250° C., and more preferably 100° C. to 140° C. The developing time is preferably 1 second to 60 seconds, more preferably 5 seconds to 30 seconds, and most preferably 10 seconds to 20 seconds.

The preferable system for thermal development is a plate-heater system. The preferable thermal development system by a plate-heater system is a system described in Japanese Patent Application Publication No. 11-133572, which is a thermal development system for obtaining visible images by contacting a thermal-developable light-sensitive material wherein a latent image has been formed with a heating means in the thermal development section. The thermal development system is characterized in that the heating means comprises a plate heater, a plurality of presser rollers are disposed facing and along a surface of the plate heater, and the thermal-developable light-sensitive material is passed between the presser rollers and the plate heater to perform thermal development. It is preferable that the plate heater is divided into two to six stages, and that the temperature of the end portion is lowered by 1 to 10° C. Such a method, also described in Japanese Patent Application Publication No. 54-30032, can exclude moisture or organic solvents contained in the thermal-developable light-sensitive material out of the system, and the deformation of

the support of the thermal-developable light-sensitive material suddenly heated can be prevented.

Although the light-sensitive material of the present invention can be exposed using any methods, a preferable light source for exposure is laser beams. The preferable laser beams for the present invention include gas laser (Ar<sup>+</sup>, He-Ne), YAG laser, dye laser, and semiconductor laser. A semiconductor laser and a second higher-harmonic-generating element can also be used. Red to infrared emitting gas or a semiconductor laser is preferable.

Laser imagers for medical use having an exposure section and a thermal development section include Fuji Medical Dry Laser Imager FM-DP L. The FM-DP L is described in Fuji Medical Review No. 8, pages 39 to 55, and these techniques can be applied to the laser imager of the thermal-developable light-sensitive material of the present invention. These techniques can also be applied to the thermal-developable light-sensitive material for the laser imager in "AD network" proposed by Fuji Medical System as a network system meeting the DICOM Standards.

The thermal-developable light-sensitive material of the present invention forms black-and-white images by silver images, and is preferably used in the thermal-developable light-sensitive material for medical diagnostics, the thermal-developable light-sensitive material for industrial photography, the thermal-developable light-sensitive material for printing, and the thermal-developable light-sensitive material for COM.

#### (Fabrication of PET Support)

Using terephthalic acid and ethylene glycol, PET having an intrinsic viscosity (IV) of 0.66 (measured in a mixed solvent of phenol and tetrachloroethane (6:4 by mass) at 25° C.) was obtained according to a normal method. This was palletized, dried at 130° C. for 4 hours, melted at 300° C., extruded through a T-die, and quenched to form a non-oriented film of a thickness after heat fixing of 175 μm.

This film was longitudinally stretched 3.3 times using rolls of different circumferential speed, and transversally stretched 4.5 times using a tenter. The temperatures for stretching were 110° C. and 130° C., respectively. Thereafter, the film was heat-fixed at 240° C. for 20 seconds, and relaxed by 4% in the transverse direction at the same temperature. Then, the portion of the film held by the chuck of the tenter was cut off, the both edges were knurled, the film was wound at 4 kg/cm<sup>2</sup> to obtain a roll of the film having a thickness of 175 μm.

#### (Corona Treatment of Surface)

The both surfaces of the support were treated using a 6-kVA solid-state corona treatment system of Piller Inc. at room temperature at 20 m/min. From the readings of current and voltage, it was known that the support was treated at 0.375 kV·A·mim/m<sup>2</sup>. The treatment frequency was 9.6 kHz, and the gap clearance between the electrode and the dielectric roller was 1.6 mm.

---

#### (Fabrication of primer coating support)

---

(1) Preparation of primer coating liquid  
Formulation (for primer-coating layer in the light-sensitive layer side)

|                                                                                                               |        |
|---------------------------------------------------------------------------------------------------------------|--------|
| Pesresin A-515GB (30% by mass solution)<br>(Takamatsu Oil & Fat)                                              | 234 g  |
| Polyethylene glycol monononyl phenyl ether<br>(average ethylene oxide number = 8.5)<br>(10% by mass solution) | 21.5 g |

-continued

| (Fabrication of primer coating support)                                                                           |        |
|-------------------------------------------------------------------------------------------------------------------|--------|
| MP-1000 (Soken Chemical & Engineering)<br>(polymer fine particles, average particle diameter: 0.4 $\mu\text{m}$ ) | 0.91 g |
| Distilled water                                                                                                   | 744 mL |
| Formulation (for first layer in back surface)                                                                     |        |
| Styrene-butadiene copolymer latex<br>(solid content: 40% by mass, styrene/butadiene mass ratio: 68/32)            | 158 g  |
| 2,4-dichloro-6-hydroxy-S-triazine, sodium salt<br>(8% by mass aqueous solution)                                   | 20 g   |
| Sodium laurylbenzenesulfonate<br>(1% by mass aqueous solution)                                                    | 10 mL  |
| Distilled water                                                                                                   | 854 mL |
| Formulation (for second layer in back surface)                                                                    |        |
| SnO <sub>2</sub> /SbO<br>(9/1 mass ratio, average particle diameter: 0.038 $\mu\text{m}$ , 17 mass % dispersion)  | 84 g   |
| Gelatin (10% by mass aqueous solution)                                                                            | 89.2 g |
| Metolose TC-5 (2% by mass aqueous solution)<br>(Shin-Etsu Chemical)                                               | 8.6 g  |
| MP-1000 (Soken Chemical & Engineering)                                                                            | 0.01 g |
| Sodium dodecylbenzenesulfonate<br>(1% by mass aqueous solution)                                                   | 10 mL  |
| NaOH (1% by mass)                                                                                                 | 6 mL   |
| Prokicell (IC <sub>1</sub> )                                                                                      | 1 mL   |
| Distilled water                                                                                                   | 805 mL |

## (Fabrication of Primer Coated Support)

After the both surfaces of the above-described biaxially oriented polyethylene terephthalate support having a thickness of 175  $\mu\text{m}$  was subjected to the above-described corona discharge treatment, one surface (light-sensitive layer side) was coated with the primer coating liquid of the above-described formulation with a wire bar so that the wet coating quantity became 6.6 mL/m<sup>2</sup> (per surface), and dried at 180° C. for 5 minutes. Then, the other surface (back face) was coated with the primer coating liquid of above-described formulation with a wire bar so that the wet coating quantity became 5.7 mL/m<sup>2</sup>, and dried at 180° C. for 5 minutes. Furthermore, the other surface (back face) was coated with the primer coating liquid of above-described formulation with a wire bar so that the wet coating quantity became 7.7 mL/m<sup>2</sup>, and dried at 180° C. for 6 minutes to fabricate a primer coated support.

## (Preparation of Back-face Coating Liquid)

## (Preparation of Fine Solid Particle Dispersion (a) of Basic Precursor)

With 220 mL of distilled water, 64 g of the basic precursor compound 11, 28 g of diphenyl sulfide, and 10 g of Demol N (surfactant, Kao Corp.) were mixed, and the mixture was subjected to bead dispersion using a sand mill (1/4-gallon sand grinder mill, Aimex) to form a fine solid particle dispersion (a) of the basic precursor having an average particle diameter of 0.2  $\mu\text{m}$ .

## (Preparation of Fine Solid Particle Dispersion of Dye)

With 305 mL of distilled water, 9.6 g of cyanine dye compound 13 and 5.8 g of sodium p-dodecylbenzenesulfonate were mixed, and the mixture was subjected to bead dispersion using a sand mill (1/4-gallon sand grinder mill, Aimex) to form a fine solid particle dispersion of the dye having an average particle diameter of 0.2  $\mu\text{m}$ .

## (Preparation of Anti-halation Coating Liquid)

Seventeen grams of gelatin, 9.6 g of polyacrylamide, 70 g of the above-described fine solid particle dispersion (a) of the basic precursor, 56 g of the above-described fine solid particle dispersion of the dye, 1.5 g of fine particles of

monodisperse polymethyl methacrylate (average particle size: 8  $\mu\text{m}$ , standard deviation of particle diameters: 0.4), 0.03 g of benzoisothiazolinone, 2.2 g of sodium polyethylenesulfonate, 0.2 g of blue dye compound 14, 3.9 g of yellow dye compound 15, and 844 mL of water were mixed to prepare an anti-halation coating.

## (Preparation of Back Face Protecting Coating)

A container was maintained at a temperature of 40° C., 50 g of gelatin, 0.2 g of sodium polystyrenesulfonate, 2.4 g of N,N-ethylenabis(vinylsulfonacetamide), 1 g of sodium t-octylphenoxyethoxyethanesulfonate, 30 mg of benzoisothiazolinone, 37 mg of a fluorine-based surfactant (F-1: N-perfluoroctylsulfonyl-N-propylalanine, potassium salt), 0.15 g of a fluorine-based surfactant (F-2: polyethylene glycol mono (N-perfluoroctylsulfonyl-N-propyl-2-aminoethyl) ether (average polymerization degree of ethylene oxide: 15)), 64 mg of a fluorine-based surfactant (F-3), 32 mg of a fluorine-based surfactant (F-4), 8.8 g of acrylic acid/ethyl acrylate copolymer (copolymerization mass ratio: 5/95), 0.6 g of Aerosol TO (American Cyanamide), 1.8 g of liquid paraffin emulsion (as liquid paraffin), and 950 mL of water were mixed to prepare a back face protecting coating liquid.

## &lt;Preparation of Silver Halide Emulsion 1&gt;

25 A liquid prepared by adding 3.1 mL of 1% by mass solution of potassium bromide, 3.5 mL of sulfuric acid of a 0.5 mole/L concentration, and 31.7 g of phthalated gelatin to 1421 mL of distilled water was maintained at a temperature of 30° C. while stirring in a stainless-steel reaction vessel, 30 solution A of 22.22 g of silver nitrate in distilled water diluted to 95.4 mL, and solution B of 15.3 g of potassium bromide and 0.8 g of potassium iodide in distilled water diluted to a volume of 97.4 mL were totally added at a constant flow rate in 45 seconds. Thereafter, 10 mL of 3.5% 35 by mass aqueous solution of hydrogen peroxide was added, and 10.8 mL of 10% by mass aqueous solution of benzimidazol was further added. Furthermore, solution C of 51.86 g of silver nitrate in distilled water diluted to 317.5 mL was totally added at a constant flow rate in 20 minutes; and 40 solution D of 2.2 g of potassium iodide in distilled water diluted to a volume of 400 mL was added by the controlled double-jet method maintaining pAg at 8.1. Hexachloroiridic (III) acid, potassium salt was totally added in a quantity ratio of  $1 \times 10^{-4}$  mole to 1 mole of silver 10 minutes after starting 45 the addition of solutions C and D. Also, an aqueous solution of potassium hexacyanoferrate (III) was added in a quantity ratio of  $3 \times 10^{-4}$  mole to 1 mole of silver 5 seconds after completing the addition of solution C. Using sulfuric acid of a 0.5 mole/L concentration, pH was adjusted to 3.8, stirring 50 was stopped, and settling, desalination, and water washing were performed. Using sodium hydroxide of a 1 mole/L concentration, pH was adjusted to 5.9, to form a silver halide dispersion of pAg of 8.0.

The above-described silver halide dispersion was maintained at a temperature of 38° C. while stirring, 5 mL of 0.34% by mass solution of 1,2-benzoisothiazoline-3-one in methanol was added, then 40 minutes later, a methanol solution of spectrally sensitizing dye A and sensitizing dye B in a mole ratio of 1:1 was added in a quantity of  $1.2 \times 10^{-3}$  60 mole as the total quantity of the sensitizing dyes A and B, and 1 minute later, the temperature was elevated to 47° C. Twenty minutes after the elevation of the temperature, a methanol solution of sodium benzenethio sulfonate was added in a quantity of  $7.6 \times 10^{-5}$  mole to 1 mole of silver, and 65 5 minutes later, the tellurium sensitizing dye B in a quantity of  $2.9 \times 10^{-4}$  mole to 1 mole of silver was added, and the dispersion was aged for 91 minutes. To the dispersion, 1.3

mL of 0.8% by mass solution of N,N'-dihydroxy-N"-diethylmelamine in methanol was added, and 4 minutes later, a methanol solution of 5-methyl-2-mercaptopbenzimidazole was added in a quantity of  $4.8 \times 10^{-3}$  mole to 1 mole of silver and a methanol solution of 1-phenyl-2-hyptyl-5-mercaptop-1,3,4-triazole was added in a quantity of  $5.4 \times 10^{-3}$  mole to 1 mole of silver, to form silver halide emulsion 1.

The particles in the prepared silver halide emulsion were silver iodide bromide particles evenly containing 3.5 mol % of iodine of an average sphere-equivalent diameter of 0.042  $\mu\text{m}$  and a coefficient of variation of the sphere-equivalent diameter of 20%. The particle size and the like were obtained from the average of 1000 particles using an electron microscope. The ratio of the {100} face of these particles was calculated to be 80% using the Kubelka-Munch method.

<Preparation of Silver Halide Emulsion 2>

Silver halide emulsion 2 was prepared in the same manner as in the preparation of silver halide emulsion 1, except that the liquid temperature in forming particles was changed from 30° C. to 47° C., solution B was changed to 15.9 g of potassium bromide dissolved in distilled water and diluted to 97.4 mL, solution D was changed to 45.8 g of potassium bromide dissolved in distilled water and diluted to 400 mL, time for adding solution C was 30 minutes, and potassium hexacyanoferrate (III) was excluded. In the same manner as in silver halide emulsion 1, precipitation, desalination, water washing, and dispersion were carried out. Furthermore, spectral sensitization and chemical sensitization, and the addition of 5-methyl-2-mercaptopbenzimidazole and 1-phenyl-2-heptyl-5-mercaptop-1,3,4-triazole were carried out in the same manner as in the preparation of silver halide emulsion 1, except that the quantity of the methanol solution of spectrally sensitizing dye A and sensitizing dye B in a mole ratio of 1:1 was changed to  $7.5 \times 10^{-4}$  mole as the total quantity of the sensitizing dyes A and B, the quantity of the tellurium sensitizing dye B to  $1.1 \times 10^{-4}$  mole to 1 mole of silver, and the quantity of 1-phenyl-2-hyptyl-5-mercaptop-1,3,4-triazole was changed to  $3.3 \times 10^{-3}$  mole to 1 mole of silver, to form silver halide emulsion 2. The emulsion particles in silver halide emulsion 2 were pure silver bromide cubic particles of an average sphere-equivalent diameter of 0.008  $\mu\text{m}$  and a coefficient of variation of the sphere-equivalent diameter of 20%.

(Preparation of Silver Halide Emulsion 3>

Silver halide emulsion 3 was prepared in the same manner as in the preparation of silver halide emulsion 1, except that the liquid temperature in forming particles was changed from 30° C. to 27° C. Also, in the same manner as in silver halide emulsion 1, precipitation, desalination, water washing, and dispersion were carried out. In the same manner as in the preparation of silver halide emulsion 1, except that the spectrally sensitizing dye A and spectrally sensitizing dye B in a mole ratio of 1:1 was changed to a solid dispersion (aqueous solution of gelatin) and the quantity was changed to  $6 \times 10^{-3}$  mole as the total quantity of the sensitizing dyes A and B, and the quantity of the tellurium sensitizing dye B to  $5.2 \times 10^{-4}$  mole to 1 mole of silver, to form silver halide emulsion 3. The emulsion particles in the silver halide emulsion 3 were silver iodide bromide particles containing 3.5 mol % of iodine of an average sphere-equivalent diameter of 0.034  $\mu\text{m}$  and a coefficient of variation of the sphere-equivalent diameter of 20%.

<Preparation of Mixed Emulsion A for Coating Liquid>

Seventy percent by mass of the silver halide emulsion 1, 15% by mass of the silver halide emulsion 2, and 15% by

mass of the silver halide emulsion 3 were dissolved, and  $7 \times 10^{-3}$  mole of benzothiazolium iodide for 1 mole of silver was added in a 1 % by mass aqueous solution. Furthermore, water was added so that the content of silver halide in 1 kg of the mixed emulsion for coating liquid became 38.2 g as silver.

<Preparation of Silver Fatty-acid Salt Dispersion>

A sodium behenate solution was obtained by mixing 87.6 kg of behenic acid (Henkel, tradename: Edenor C22-85R), 423 L of distilled water, 49.2 L of a 5 mole/L aqueous solution of NaOH, and 120 L of tert-butanol, and stirring at 75° C. for 1 hour to allow to react. Separately, 206.2 L of an aqueous solution containing 40.4 Kg of silver nitrate (pH 4.0) was prepared, and maintained at a temperature of 10° C. 15 A reaction vessel containing 635 L of distilled water and 30 L of tert-butanol was maintained at a temperature of 30° C., and the total quantity of the above-described sodium behenate solution and the total quantity of the aqueous solution of silver nitrate were added stirring well in 93 minutes 15 seconds and 90 minutes, respectively. In this time, only the aqueous solution of silver nitrate was added for 11 minutes from the start of adding, then, the addition of the sodium behenate solution was started, and only the sodium behenate solution was for 14 minutes 15 seconds after the completion of adding the aqueous solution of silver nitrate. The temperature in the reaction vessel at this time was 30° C., and the ambient temperature was controlled so that the liquid temperature is maintained constant. The piping for adding the sodium behenate solution was warmed by circulating warm water in the outer pipe of the double-pipe system, and the liquid temperature at the outlet of the adding nozzle was controlled to be 75° C. The piping for adding the aqueous solution of silver nitrate was warmed by circulating cold water in the outer pipe of the double-pipe system. The location of adding the sodium behenate solution and the location of the aqueous solution of silver nitrate were symmetrical about the axis of stirring, and adjusted to the height so as not to contact the reaction liquid.

After completing the addition of the sodium behenate solution, the temperature of the solution was maintained at the same temperature stirring for 20 minutes, and elevated to 35° C. in 30 minutes, and the solution was aged for 210 minutes. Immediately after the completion of aging, pure water was added in the tank to stop aging, the solution was 45 transferred from the feeding kettle by head pressure or using a pump, the solid matter was filtered by centrifugal filtration, and washed with water until the conductivity of the filtrate becomes 30  $\mu\text{S}/\text{cm}$ . Thus, the fatty salt of silver was obtained. The obtained solid matter was stored as wet cake 50 (solid content: 45% by mass) without drying.

The form of the obtained silver behenate particles observed by electron microscopic photography was flake crystals having average values of  $a=0.14 \mu\text{m}$ ,  $b=0.4 \mu\text{m}$ ,  $c=0.6 \mu\text{m}$ ; an average aspect ratio of 5.2; an sphere-equivalent diameter of 0.52  $\mu\text{m}$  and a coefficient of variation of the sphere-equivalent diameter of 15%. (a, b, and c are defined herein.)

To the wet cake equivalent to 260 kg of the dry solid, 19.3 kg of polyvinyl alcohol (trade name: PVA-217) and water 60 were added to make the total quantity of 1000 kg, the mixture was made to be slurry using a dissolver blade, and preliminarily dispersed with a pipe-line mixer (MIZUHO, PM-10).

Next, the preliminarily dispersed stock slurry was treated 65 3 times with a dispersing machine (trade name: Micro Fluidizer M-610, Microfluidex International Corporation, using a Z-type interaction chamber) of which pressure was

adjusted to 1260 kg/cm<sup>2</sup>, to form silver behenate dispersion. The dispersion temperature of 18° C. was maintained by furnishing coiled heat exchangers before and after the interaction chamber, respectively, and controlling the temperature of the coolant.

<Preparation of Reducer-1 Dispersion>

To 10 kg of the reducer-1 (1,1-bis(2-hydroxy-3,5-dimethylphenyl)-3,5,5-trimethylhexane) and 10 kg of a 20% by mass aqueous solution of modified polyvinyl alcohol (KURARAY, POVAL MP203), 16 kg of water was mixed, and the mixture was stirred well to form a slurry. The slurry was pumped with a diaphragm pump to a horizontal sand mill packed with zirconia beads of an average diameter of 0.5 mm (IMEX, UVM-2), whereby it was dispersed for 3 hours 30 minutes, then, 0.2 g of benzoisothiazolinone sodium salt and water were added to adjust so that the concentration of the reducer became 25% by mass to form a reducer-1 dispersion. The reducer particles in thus obtained reducer dispersion had a median diameter of 0.42  $\mu\text{m}$  and a maximum particle diameter of 2.0  $\mu\text{m}$  or smaller. The obtained reducer dispersion was filtered with a polypropylene filter of a pore diameter of 10.0  $\mu\text{m}$  to remove foreign matter, such as dust, and stored.

<Preparation of Reducer-2 Dispersion>

To 10 kg of the reducer-2 (2,2'-isobutylidene-bis-(4,6-dimethylphenol)) and 10 kg of a 20% by mass aqueous solution of modified polyvinyl alcohol (KURARAY, POVAL MP203), 16 kg of water was mixed, and the mixture was stirred well to form a slurry. The slurry was pumped with a diaphragm pump to a horizontal sand mill packed with zirconia beads of an average diameter of 0.5 mm (IMEX, UVM-2), whereby it was dispersed for 3 hours 30 minutes, then, 0.2 g of benzoisothiazolinone sodium salt and water were added to adjust so that the concentration of the reducer became 25% by mass to form a reducer-2 dispersion. The reducer particles in thus obtained reducer dispersion had a median diameter of 0.38  $\mu\text{m}$  and a maximum particle diameter of 2.0  $\mu\text{m}$  or smaller. The obtained reducer dispersion was filtered with a polypropylene filter of a pore diameter of 10.0  $\mu\text{m}$  to remove foreign matter, such as dust, and stored.

<Preparation of Reducer Complex-3 Dispersion>

To 10 kg of the reducer complex-3 (1:1 complex of 2,2'-methylene-bis(4-ethyl-6-tert-butylphenol) and hydrogen linkable compound-1 (triphenylphosphine oxide)), 0.12 kg of triphenylphosphine oxide, and 16 kg of a 10% by mass aqueous solution of modified polyvinyl alcohol (KURARAY, POVAL MP203), 7.2 kg of water was mixed, and the mixture was stirred well to form a slurry. The slurry was pumped with a diaphragm pump to a horizontal sand mill packed with zirconia beads of an average diameter of 0.5 mm (IMEX, UVM-2), whereby it was dispersed for 4 hours 30 minutes, then, 0.2 g of benzoisothiazolinone sodium salt and water were added to adjust so that the concentration of the reducer became 25% by mass to form a reducer complex-3 dispersion. The reducer particles in thus obtained reducer dispersion had a median diameter of 0.46  $\mu\text{m}$  and a maximum particle diameter of 1.6  $\mu\text{m}$  or smaller. The obtained reducer dispersion was filtered with a polypropylene filter of a pore diameter of 3.0  $\mu\text{m}$  to remove foreign matter, such as dust, and stored.

<Preparation of Reducer-4 Dispersion>

To 10 kg of the reducer-4 (2,2'-methylene-bis(4-ethyl-6-tert-butylphenol)) and 20 kg of a 10% by mass aqueous solution of modified polyvinyl alcohol (KURARAY, POVAL MP203), 6 kg of water was mixed, and the mixture was stirred well to form a slurry. The slurry was pumped

with a diaphragm pump to a horizontal sand mill packed with zirconia beads of an average diameter of 0.5 mm (IMEX, UVM-2), whereby it was dispersed for 3 hours 30 minutes, then, 0.2 g of benzoisothiazolinone sodium salt and water were added to adjust so that the concentration of the reducer became 25% by mass to form a reducer-4 dispersion. The reducer particles in thus obtained reducer dispersion had a median diameter of 0.40  $\mu\text{m}$  and a maximum particle diameter of 1.5  $\mu\text{m}$  or smaller. The obtained reducer dispersion was filtered with a polypropylene filter of a pore diameter of 3.0  $\mu\text{m}$  to remove foreign matter, such as dust, and stored.

<Preparation of Reducer-5 Dispersion>

To 10 kg of the reducer-5 (2,2'-methylene-bis(4-methyl-6-tert-butylphenol)) and 20 kg of a 10% by mass aqueous solution of modified polyvinyl alcohol (KURARAY, POVAL MP203), 6 kg of water was mixed, and the mixture was stirred well to form a slurry. The slurry was pumped with a diaphragm pump to a horizontal sand mill packed with zirconia beads of an average diameter of 0.5 mm (IMEX, UVM-2), whereby it was dispersed for 3 hours 30 minutes, then, 0.2 g of benzoisothiazolinone sodium salt and water were added to adjust so that the concentration of the reducer became 25% by mass to form a reducer-5 dispersion. The reducer particles in thus obtained reducer dispersion had a median diameter of 0.38  $\mu\text{m}$  and a maximum particle diameter of 1.5  $\mu\text{m}$  or smaller. The obtained reducer dispersion was filtered with a polypropylene filter of a pore diameter of 3.0  $\mu\text{m}$  to remove foreign matter, such as dust, and stored.

<Preparation of Hydrogen Linkable Compound-2 Dispersion>

To 10 kg of the hydrogen linkable compound-2 (tri(4-tert-butylphenyl)phosphine oxide) and 20 kg of a 10% by mass aqueous solution of modified polyvinyl alcohol (KURARAY, POVAL MP203), 10 kg of water was mixed, and the mixture was stirred well to form a slurry. The slurry was pumped with a diaphragm pump to a horizontal sand mill packed with zirconia beads of an average diameter of 0.5 mm (IMEX, UVM-2), whereby it was dispersed for 3 hours 30 minutes, then, 0.2 g of benzoisothiazolinone sodium salt and water were added to adjust so that the concentration of the reducer became 22% by mass to form a hydrogen linkable compound-2 dispersion. The reducer particles in thus obtained reducer dispersion had a median diameter of 0.35  $\mu\text{m}$  and a maximum particle diameter of 1.5  $\mu\text{m}$  or smaller. The obtained reducer dispersion was filtered with a polypropylene filter of a pore diameter of 3.0  $\mu\text{m}$  to remove foreign matter, such as dust, and stored.

<Preparation of Organic Polyhalogen Compound-1 Dispersion>

To 10 kg of the organic polyhalogen compound-1 (2-tribromomethane sulfonyl naphthalene), 10 kg of a 20% by mass aqueous solution of modified polyvinyl alcohol (KURARAY, POVAL MP203), and 0.4 kg of a 20% by mass aqueous solution of sodium triisopropylnaphthalenesulfonate, 16 kg of water was mixed, and the mixture was stirred well to form a slurry. The slurry was pumped with a diaphragm pump to a horizontal sand mill packed with zirconia beads of an average diameter of 0.5 mm (IMEX, UVM-2), whereby it was dispersed for 5 hours, then, 0.2 g of benzoisothiazolinone sodium salt and water were added to adjust so that the concentration of the organic polyhalogen compound became 23.5% by mass to form an organic polyhalogen compound-1 dispersion. The organic polyhalogen compound particles in thus obtained organic polyhalogen compound dispersion had a median

diameter of  $0.36\text{ }\mu\text{m}$  and a maximum particle diameter of  $2.0\text{ }\mu\text{m}$  or smaller. The obtained organic polyhalogen compound dispersion was filtered with a polypropylene filter of a pore diameter of  $10.0\text{ }\mu\text{m}$  to remove foreign matter, such as dust, and stored.

<Preparation of Organic Polyhalogen Compound-2 Dispersion>

To 10 kg of the organic polyhalogen compound-2 (tribromomethane sulfonyl benzene), 10 kg of a 20% by mass aqueous solution of modified polyvinyl alcohol (KURARAY, POVAL MP203), and 0.4 kg of a 20% by mass aqueous solution of sodium triisopropylnaphthalenesulfonate, 14 kg of water was mixed, and the mixture was stirred well to form a slurry. The slurry was pumped with a diaphragm pump to a horizontal sand mill packed with zirconia beads of an average diameter of 0.5 mm (IMEX, UVM-2), whereby it was dispersed for 5 hours, then, 0.2 g of benzoisothiazolinone sodium salt and water were added to adjust so that the concentration of the organic polyhalogen compound became 26% by mass to form an organic polyhalogen compound-2 dispersion. The organic polyhalogen compound particles in thus obtained organic polyhalogen compound dispersion had a median diameter of  $0.41\text{ }\mu\text{m}$  and a maximum particle diameter of  $2.0\text{ }\mu\text{m}$  or smaller. The obtained organic polyhalogen compound dispersion was filtered with a polypropylene filter of a pore diameter of  $10.0\text{ }\mu\text{m}$  to remove foreign matter, such as dust, and stored.

<Preparation of Organic Polyhalogen Compound-3 Dispersion>

To 10 kg of the organic polyhalogen compound-3 (N-butyl-3-tribromomethanesulfonyl benzamide), 10 kg of a 20% by mass aqueous solution of modified polyvinyl alcohol (KURARAY, POVAL MP203), and 0.4 kg of a 20% by mass aqueous solution of sodium triisopropylnaphthalenesulfonate, 8 kg of water was mixed, and the mixture was stirred well to form a slurry. The slurry was pumped with a diaphragm pump to a horizontal sand mill packed with zirconia beads of an average diameter of 0.5 mm (IMEX, UVM-2), whereby it was dispersed for 5 hours, then, 0.2 g of benzoisothiazolinone sodium salt and water were added to adjust so that the concentration of the organic polyhalogen compound becomes 25% by mass to form an organic polyhalogen compound-3 dispersion. The organic polyhalogen compound particles in thus obtained organic polyhalogen compound dispersion had a median diameter of  $0.36\text{ }\mu\text{m}$  and a maximum particle diameter of  $1.5\text{ }\mu\text{m}$  or smaller. The obtained organic polyhalogen compound dispersion was filtered with a polypropylene filter of a pore diameter of  $3.0\text{ }\mu\text{m}$  to remove foreign matter, such as dust, and stored.

<Preparation of Phthalazine Compound-1 Solution>

Eight kilograms of modified polyvinyl alcohol MP203 (KURARAY) was dissolved in 174.57 kg of water, then 3.15 kg of a 20% by mass aqueous solution of sodium triisopropylnaphthalenesulfonate and 14.28 kg of a 70% by mass aqueous solution of phthalazine compound-1 (6-isopropylphthalazine) were added to prepare 5% by mass solution of phthalazine compound-1.

<Preparation of Mercapto Compound-1 Solution>

Seven grams of mercapto compound-1 (1-(3-sulfophenyl)-5-mercaptop tetrazole sodium salt) was dissolved in 993 g of water to prepare 0.7% by mass aqueous solution of mercapto compound-1.

<Preparation of Pigment-1 Dispersion>

To 64 g of C. I. Pigment Blue 60 and 6.4 g of Kao DEMOL N, 250 g of water was added, and the mixture was stirred well to form slurry. Together the slurry, 800 g of zirconia beads of an average diameter of 0.5 mm were fed in a vessel, and dispersed for 25 hours with a dispersing machine (1/4G Sand Grinder Mill, IMEX) to form a

pigment-1 dispersion. The pigment particles in thus obtained pigment dispersion had an average particle diameter of  $0.21\text{ }\mu\text{m}$ .

<Preparation of SBR Latex Emulsion>

SBR latex of a Tg of  $23^\circ\text{ C.}$  was prepared as follows: 5 Using ammonium persulfate as a polymerization initiator, and an anionic surfactant as an emulsifier, 70.5 parts by mass of styrene, 26.5 parts by mass of butadiene, and 3 parts by mass of acrylic acid were undergone emulsion polymerization, and aged at  $80^\circ\text{ C.}$  for 8 hours. Thereafter, 10 the emulsion was cooled to  $40^\circ\text{ C.}$ ; the pH was adjusted to 7.0 using ammonia water; and Sandet BL (Sanyo Chemical Industries) was added to a concentration of 0.22%. Next, a 15 5% aqueous solution of sodium hydroxide was added to pH 8.3, and furthermore, the pH was adjusted to 8.4 using ammonia water. The mole ratio of  $\text{Na}^+$  ions and  $\text{NH}_4^+$  ions used in this time was 1:2.3. Furthermore, 0.15 mL of a 7% aqueous solution of benzoisothiazolinone sodium salt was added to 1 kg of the emulsion to prepare an SBR latex emulsion.

(SBR latex: St (70.5)-Bu (26.5)-AA (3)-latex) Tg:  $23^\circ\text{ C.}$

Average particle diameter:  $0.1\text{ }\mu\text{m}$ ; concentration: 43% by mass; equilibrium water content at  $25^\circ\text{ C.}$ , 60% RH: 0.6% by mass; ionic conductivity: 4.2 mS/cm (measured using DKK-TOA conductivity meter CM-30S for the latex stock emulsion (43% by mass) at  $25^\circ\text{ C.}$ ); pH: 8.4

20 SBR latex of different Tg was prepared by the same manner except for changing the contents of styrene and butadiene.

<Preparation of Emulsion Layer (Light-sensitive Layer) Coating Liquid-1>

The emulsion layer coating liquid prepared by sequentially adding 1000 g of the dispersion of fatty-acid salt of silver obtained as described above, 125 mL of water, 113 g of the dispersion of the reducer-1, 91 g of the dispersion of the reducer-2, 27 g of the dispersion of the pigment-1, 82 g of the dispersion of the organic polyhalogen compound-1, 40 g of the dispersion of the organic polyhalogen compound-2, 173 g of the solution of the phthalazine compound-1, 1082 g of the SBR latex (Tg:  $20.5^\circ\text{ C.}$ ) emulsion, and 9 g of the aqueous solution of the mercapto compound-1, adding 158 g of the silver halide mixed emulsion A immediately before 25 coating, and mixing well was transferred as it is to a coating die and applied.

The viscosity of the emulsion layer coating liquid measured at  $40^\circ\text{ C.}$  using a B-viscometer (Tokyo Keiki) was 85 mPa·s (No. 1 rotor, 60 rpm).

45 The viscosities of the coating liquid at  $25^\circ\text{ C.}$  measured using an RFS Fluid Spectrometer manufactured by Rheometrics Far East at shear rates of  $0.1\text{ s}^{-1}$ ,  $1\text{ s}^{-1}$ ,  $10\text{ s}^{-1}$ ,  $100\text{ s}^{-1}$ , and  $1000\text{ s}^{-1}$  were 1500 mPa·s, 220 mPa·s, 70 mPa·s, 40 mPa·s, and 20 mPa·s, respectively.

<Preparation of Emulsion Layer (Light-sensitive Layer) Coating Liquid-2>

The emulsion layer coating liquid prepared by sequentially adding 1000 g of the dispersion of fatty-acid salt of silver obtained as described above, 104 mL of water, 30 g of the dispersion of the pigment-1, 21 g of the dispersion of the organic polyhalogen compound-2, 69 g of the dispersion of the organic polyhalogen compound-3, 173 g of the solution of the phthalazine compound-1, 1082 g of the SBR latex (Tg:  $23^\circ\text{ C.}$ ) emulsion, 258 g of the dispersion of the reducer complex-3, and 9 g of the solution of the mercapto compound-1, adding 110 g of the silver halide mixed emulsion A immediately before coating, and mixing well was transferred as it is to a coating die and applied.

<Preparation of Emulsion Layer (Light-sensitive Layer) Coating Liquid-3>

60 The emulsion layer coating liquid prepared by sequentially adding 1000 g of the dispersion of fatty-acid salt of silver obtained as described above, 95 mL of water, 73 g of

the dispersion of the reducer-4, 68 g of the dispersion of the reducer-5, 30 g of the dispersion of the pigment-1, 21 g of the dispersion of the organic polyhalogen compound-2, 69 g of the dispersion of the organic polyhalogen compound-3, 173 g of the solution of the phthalazine compound-1, 1082 g of the core-shell type SBR latex (core Tg: 20° C./shell Tg: 30° C.=70/30) emulsion, 124 g of the dispersion of the hydrogen-linkable compound-2, and 9 g of the aqueous solution of the mercapto compound-1, adding 110 g of the silver halide mixed emulsion A immediately before coating, and mixing well was transferred as it is to a coating die and applied.

<Preparation of Intermediate Emulsion Layer Coating Liquid>

The intermediate emulsion layer coating liquid prepared by mixing 772 g of a 10% by mass aqueous solution of polyvinyl alcohol PVA-205 (KURARAY), 5.3 g of the dispersion of pigment, 226 g of a 27.5% by mass emulsion of a methyl methacrylate/styrene/butyl acrylate/hydroxyethyl methacrylate/acrylic acid copolymer (copolymerization ratio by mass: 64/9/20/5/2) latex, 2 mL of a 5% by mass aqueous solution of Aerosol TO (American Cyanamide), 10.5 mL of a 20% by mass aqueous solution of di ammonium phthalate, and adding water to make the total quantity 880 g, adjusting the pH to 7.5 with NaOH was transferred to a coating die so as to be 10 mL/m<sup>2</sup>.

The viscosity of the coating liquid measured at 40° C. using a B-viscometer was 21 mPa·s (No. 1 rotor, 60 rpm).

<Preparation of First Emulsion Protecting Layer Coating Liquid>

The coating liquid prepared by dissolving 64 g of inert gelatin in water, adding 80 g of a 27.5% by mass emulsion of a methyl methacrylate/styrene/butyl acrylate/hydroxyethyl methacrylate/acrylic acid copolymer (copolymerization ratio by mass: 64/9/20/5/2) latex, 23 mL of a 10% by mass methanol solution of phthalic acid, 23 mL of a 10% by mass aqueous solution of 4-methylphthalic acid, 28 mL of sulfuric acid of a concentration of 0.5 mole/L, 5 mL of a 5% by mass aqueous solution of Aerosol TO (American Cyanamide), 0.5 g of phenoxy ethanol, and 0.1 g of benzoisothiazolinone, adding water to make the total quantity 750 g, and mixing 26 mL of a 4% by mass solution of chrome alum with a static mixer immediately before coating was transferred to a coating die so as to be 18.6 mL/m<sup>2</sup>.

The viscosity of the coating liquid measured at 40° C. using a B-viscometer was 17 mPa·s (No. 1 rotor, 60 rpm).

<Preparation of Second Emulsion Protecting Layer Coating Liquid>

The coating liquid for surface-protecting layer prepared by dissolving 80 g of inert gelatin in water, adding 102 g of a 27.5% by mass emulsion of a methyl methacrylate/styrene/butyl acrylate/hydroxyethyl methacrylate/acrylic acid copolymer (copolymerization ratio by mass: 64/9/20/5/2) latex, 3.2 mL of a 5% by mass solution of a fluorine-based surfactant (F-1: N-perfluorooctylsulfonyl-N-propylglycine potassium salt), 32 mL of a 2% by mass aqueous solution of a fluorine-based surfactant (F-2: polyethyleneglycol mono (N-perfluorooctylsulfonyl-N-propyl-2-aminoethyl)ether (average degree of polymerization of ethylene oxide=15), 23 mL of a 5% by mass solution of Aerosol TO (American Cyanamide), 4 g of fine particles of polymethyl methacrylate (average particle diameter: 0.7 μm), 21 g of fine particles of polymethyl methacrylate (average particle diameter: 4.5 μm), 1.6 g of 4-methyl phthalic acid, 4.8 g of phthalic acid, 44 mL of sulfuric acid of a concentration of 0.5 mole/L, and 10 mg of benzoisothiazolinone, adding water to make the total quantity 650 g, and mixing 445 mL of an aqueous solution containing 4% by mass chrome alum and 0.67% by

mass phthalic acid with a static mixer immediately before coating was transferred to a coating die so as to be 8.3 mL/m<sup>2</sup>.

The viscosity of the coating liquid measured at 40° C. using a B-viscometer was 9 mPa·s (No. 1 rotor, 60 rpm).

<Preparation of Thermal-developable Light-sensitive Material-1>

The back-face side of the above-described primer support was coated with the anti-halation layer coating liquid so that the coating quantity of the solid matter of the fine solid particle dye became 0.04 g/m<sup>2</sup>, and was simultaneously coated with the back-face protecting layer coating liquid so that the gelatin quantity became 1.7 g/m<sup>2</sup>, dried to form a back layer. The surface opposite to the back face, from the primer surface, was simultaneously coated with the emulsion layer, the intermediate layer, the first protecting layer, and the second protecting layer in this order in slide-bead application method to form the sample of the thermal-developable light-sensitive material. In this time, the temperatures of the emulsion layer and the intermediate layer, the first protecting layer, and the second protecting layer were adjusted to 31° C., 36° C., and 37° C., respectively.

The coating quantity (g/m<sup>2</sup>) of each compound as the emulsion layer is as follows:

|                                 |       |
|---------------------------------|-------|
| Silver behenate                 | 6.19  |
| Reducer-1                       | 0.67  |
| Reducer-2                       | 0.54  |
| Pigment (C. I. Pigment Blue 60) | 0.032 |
| Polyhalogen compound-1          | 0.46  |
| Polyhalogen compound-2          | 0.25  |
| Phthalazine compound-1          | 0.21  |
| SBR latex                       | 11.1  |
| Mercapto compound-1             | 0.002 |
| Silver halide (as Ag)           | 0.145 |

Coating and drying conditions were as follows:

Coating was performed at a speed of 160 m/min, a distance between the end of the coating die and the support of 0.10 mm and 0.30 mm, and the pressure of the reduced-pressure chamber was set 196 Pa to 882 Pa lower than atmospheric pressure. The support was ionized with ion wind before coating.

In the following chilling-zone, the coating liquid was cooled with the air of a dry-bulb temperature between 10° C. and 20° C., then transferred without contacting, and dried in a helical air cushion dryer with the dry air of a dry-bulb temperature between 23° C. and 45° C. and a wet-bulb temperature between 15° C. and 21° C.

After drying, the humidity was adjusted to 40% RH to 60% RH at 25° C., and the film surface was heated to a temperature between 70° C. and 90° C. After heating, the film surface was cooled to 25° C.

The mat degree of the formed thermal-developable light-sensitive material was a Beck flatness of 550 seconds on the surface of the light-sensitive layer, and 130 seconds on the back face. The pH measured on the film surface of the light-sensitive layer surface side was 6.0.

<Preparation of Thermal-developable Light-sensitive Material-2>

Thermal-developable light-sensitive material-2 was prepared in the same manner as the thermal-developable light-sensitive material-1, except that the emulsion layer coating liquid-1 was changed to the emulsion layer coating liquid-2, and the yellow dye compound 15 was excluded from the anti-halation layer.

The coating quantity (g/m<sup>2</sup>) of each compound as the emulsion layer in this time is as follows:

|                                 |       |
|---------------------------------|-------|
| Silver behenate                 | 6.19  |
| Pigment (C. I. Pigment Blue 60) | 0.036 |
| Polyhalogen compound-2          | 0.13  |
| Polyhalogen compound-3          | 0.41  |
| Phthalazine compound-1          | 0.21  |
| SBR latex                       | 11.1  |
| Reducer complex-3               | 1.54  |
| Mercapto compound-1             | 0.002 |
| Silver halide (as Ag)           | 0.10  |

**<Preparation of Thermal-developable Light-sensitive Material-3>**

Thermal-developable light-sensitive material-3 was prepared in the same manner as the thermal-developable light-sensitive material-1, except that the emulsion layer coating liquid-1 was changed to the emulsion layer coating liquid-3; the yellow dye compound 15 was excluded from the anti-halation layer; fluorine-based surfactants F-1, F-2, F-3, and F-4 in the second protecting layer and the back-face protecting layer were changed to fluorine-based surfactants F-5, F-6, F-7, and F-8 of the same masses, respectively.

The coating quantity (g/m<sup>2</sup>) of each compound as the emulsion layer in this time is as follows:

|                                 |       |
|---------------------------------|-------|
| Silver behenate                 | 5.57  |
| Pigment (C. I. Pigment Blue 60) | 0.032 |
| Reducer-4                       | 0.40  |
| Reducer-5                       | 0.36  |
| Polyhalogen compound-2          | 0.12  |
| Polyhalogen compound-3          | 0.37  |
| Phthalazine compound-1          | 0.19  |
| SBR latex                       | 10.0  |
| Hydrogen-bondable compound-2    | 0.59  |
| Mercapto compound-1             | 0.002 |
| Silver halide (as Ag)           | 0.09  |

**(Evaluation of Photographic Performance)**

With a Fuji Medical Dry Laser Imager FM-DPL (incorporating a 660-nm semiconductor laser of a maximum output of 60 mW (IIIB), a photographic material was exposed and heat-developed (total of 24 seconds by four panel heaters set to 112° C., 119° C., 121° C., and 121° C.), and the obtained image was evaluated with a photographic densitometer.

**EXAMPLES**

Next, examples of a method for drying the coating film for a thermal-developable light-sensitive material of the present invention will be described.

A slide-bead applicator was used as the applicator in the coating process, and the support was coated with four types of coating liquids, including the coating liquid prepared in the above-described <Preparation of emulsion layer (light-sensitive layer) coating liquid> simultaneously at a coating speed of 150 m/min. In this time, the quantities of coating

liquids supplied to the applicator were controlled so that the thickness of four layers of the coating liquids with which the support was coated became 80  $\mu$ m.

The process of drying coating films comprised a chilling-zone step, a PAC drying step and an HAC drying step. The length (from the inlet to the outlet) of the chilling-zone step was 50 m, and the retention time at the above-described coating speed was 20 seconds. The length (from the inlet to the outlet) of the PAC drying step was 100 m, the length (from the inlet to the outlet) of the HAC drying step was 600 m, and the total of the drying process in the non-contacting state was set to be 700 m. The retention times in this case according to the above-described coating speed were 40 seconds in the PAC drying step and 240 seconds (4 minutes) in the HAC drying step.

A dual system was used in the HAC drying step, and the support after the HAC drying step was heat-treated for manufacturing the thermal-developable light-sensitive material, then wound with a winder. In Table 1, for example, “40→30° C.” in the “D.B.” column in the “Example 1” row means that the dry-bulb temperature in the first HAC drying step is 40° C., and the dry-bulb temperature in the second HAC drying step is 30° C.

The photographic sensitivity of each sample of Examples 1 to 3 manufactured by changing the dry-bulb temperature in the chilling-zone step, the dry-bulb temperature and wet-bulb temperature, and time from application to the dry point in the PAC drying step and the HAC drying step as in Table 1, was evaluated.

The evaluation criteria in Table 1 were E (excellent photographic performance), G (good photographic performance), and P (poor photographic performance), and the samples of evaluated as G or above were deemed to pass the test.

Examples 1 to 3 in Table 1 are cases where all the conditions of the method for drying the coating film for the thermal-developable light-sensitive material of the present invention are satisfied. Also, Examples 1 and 3 are cases where dry-bulb and wet-bulb temperatures are gradually lowered as the coating film is conveyed from the inlet of the PAC drying step toward the outlet of the HAC drying step. Whereas, Example 2 is the case where dry-bulb and wet-bulb temperatures in the first stage of the HAC drying step are higher than dry-bulb and wet-bulb temperatures in the PAC drying step.

Comparative Example 1 is the case where the drying process comprised only a chilling-zone step and an HAC drying step, and the length of the HAC drying step was 700 m.

Comparative Example 2 is the case where the drying process comprised a chilling-zone step, a PAC drying step, and an HAC drying step; however, dry-bulb temperatures in the PAC drying step and the HAC drying step were out of the range between 25° C. and 100° C. of the present invention, and time from application to the dry point was beyond 300 seconds of the present invention.

TABLE 1

| Example | Chilling-zone | PAC process |        | HAC process |           | Time between coating and dry point (seconds) | Evaluation of photographic performance |
|---------|---------------|-------------|--------|-------------|-----------|----------------------------------------------|----------------------------------------|
|         |               | D.B.        | W.B.   | D.B.        | W.B.      |                                              |                                        |
| 1       | 15° C.        | 40° C.      | 20° C. | 40→30° C.   | 23→20° C. | 200 sec.                                     | E                                      |
| 2       | 20° C.        | 30° C.      | 15° C. | 50→30° C.   | 25→18° C. | 170 sec.                                     | G                                      |
| 3       | 10° C.        | 50° C.      | 25° C. | 30→25° C.   | 20→16° C. | 190 sec.                                     | E                                      |

TABLE 1-continued

| Chilling-zone       | PAC process |                  | HAC process    |                     | Time between coating and dry point (seconds) | Evaluation of photographic performance |        |
|---------------------|-------------|------------------|----------------|---------------------|----------------------------------------------|----------------------------------------|--------|
|                     | D.B.        | D.B.             | W.B.           | D.B.                | W.B.                                         |                                        |        |
| Comparative example | 1<br>2      | 15° C.<br>20° C. | None<br>20° C. | 40→30° C.<br>13° C. | 23→20° C.<br>20° C.                          | 200 sec.<br>320 sec.                   | P<br>P |

As seen from the results shown in Table 1, all the photographic performances of Examples 1 to 3, all of which satisfied the conditions of the method for drying the coating film for the thermal-developable light-sensitive material of the present invention, passed the test. Although not shown in Table 1, the surface conditions of the coating films after drying of Examples 1 to 3 were excellent. The evaluation of the photographic performances of Examples 1 and 3, wherein dry-bulb and wet-bulb temperatures are gradually lowered as the coating film was conveyed from the inlet of the PAC drying step toward the outlet of the HAC drying step was E, which was better than the evaluation of the photographic performances of Example 2 of G, wherein dry-bulb and wet-bulb temperatures in the first stage of the HAC drying step were higher than dry-bulb and wet-bulb temperatures in the PAC drying step.

In Comparative Example 1 wherein the PAC drying step was omitted from the drying process including a chilling-zone step, a PAC drying step, and an HAC drying step, a little liquid scattering was observed in the HAC drying step, and the surface conditions of the coating film became poor. The photographic performance was also P. It was considered, therefore, the drying process of the coating film for the thermal-developable light-sensitive material required three steps of a chilling-zone step, a PAC drying step, and an HAC drying step.

Also the photographic performance of Comparative Example 2, wherein dry-bulb temperatures in the PAC drying step and the HAC drying step were out of the range between 25° C. and 100° C. of the present invention, and time from application to the dry point was beyond 300 seconds or below of the present invention, was evaluated as P. From this, it is the essential condition that the drying process of the coating film for the thermal-developable light-sensitive material comprises three steps of a chilling-zone step, a PAC drying step, and an HAC drying step, and it is required to set the dry-bulb temperature, the wet-bulb temperature, and time from application to the dry point adequately.

As described above, according to the method for drying the coating film for the thermal-developable light-sensitive material of the present invention, liquid scattering during drying due to the air for drying the coating film for the thermal-developable light-sensitive material can be prevented, and good surface conditions of the coating film and good photographic performance can be achieved.

It should be understood, however, that there is no intention to limit the invention to the specific forms disclosed, but on the contrary, the invention is to cover all modifications, alternate constructions and equivalents falling within the spirit and scope of the invention as expressed in the appended claims.

What is claimed is:

1. A method for drying, with drying air in a drying process, a coating film in manufacture of thermal-developable light-sensitive material formed by coating with

a coating liquid that contains an organic silver salt, a reducer for silver ions, a polymer latex, and silver halide particles to a support being conveyed in a coating process, wherein: the drying process comprises:

a chilling-zone step for cooling the coating film with cold air;

a plane air cushion drying step for a first-stage drying of the coating film in a non-contact state while floating and supporting the support by supplying a hot drying air of a predetermined wind velocity to both sides of the support;

a helical air cushion drying step for a second-stage drying of the coating film in a non-contact state while helically winding the support around a circumferential surface of a cylinder and floating and supporting the support by supplying the hot drying air from the circumferential surface of the cylinder to the coating film.

2. The method according to claim 1, wherein a speed of the coating is set within a range between 100 m/minute and 300 m/minute.

3. The method according to claim 1, wherein, in the chilling-zone, a dry-bulb temperature is set within a range between 5° C. and 50° C.; and in the constant-rate period of drying during the first-stage drying and the second-stage drying, the dry-bulb temperature is set within a range between 25° C. and 100° C. and higher than the dry-bulb temperature in the chilling-zone, and the wet-bulb temperature is set within a range between 10° C. and 50° C.

4. The method according to claim 3, wherein a speed of the coating is set within a range between 100 m/minute and 300 m/minute.

5. The method according to claim 3, wherein the dry-bulb temperature and the wet-bulb temperature are gradually lowered as the support is conveyed from an entrance side of the plane air cushion drying step toward an exit side of the helical air cushion drying step.

6. The method according to claim 5, wherein a speed of the coating is set within a range between 100 m/minute and 300 m/minute.

7. The method according to claim 1, wherein the wind velocity of the drying air in the plane air cushion drying step is set between 20 m/second and 30 m/second.

8. The method according to claim 7, wherein a speed of the coating is set within a range between 100 m/minute and 300 m/minute.

9. The method according to claim 7, wherein, in the chilling-zone, a dry-bulb temperature is set within a range between 5° C. and 50° C.; and in the constant-rate period of drying during the first-stage drying and the second-stage drying, the dry-bulb temperature is set within a range between 25° C. and 100° C. and higher than the dry-bulb temperature in the chilling-zone, and the wet-bulb temperature is set within a range between 10° C. and 50° C.

10. The method according to claim 9, wherein a speed of the coating is set within a range between 100 m/minute and 300 m/minute.

11. The method according to claim 9, wherein the dry-bulb temperature and the wet-bulb temperature are gradually lowered as the support is conveyed from an entrance side of the plane air cushion drying step toward an exit side of the helical air cushion drying step.

12. The method according to claim 11, wherein a speed of the coating is set within a range between 100 m/minute and 300 m/minute.

13. The method according to claim 1, wherein a drying point of the coating film is present within 300 seconds from the coating.

14. The method according to claim 13, wherein a speed of the coating is set within a range between 100 m/minute and 300 m/minute.

15. The method according to claim 13, wherein a <sup>15</sup> humidity-controlling time from the drying point of the

coating film until the support is wound by a winding device is set within a range between 10 seconds and 200 seconds.

16. The method according to claim 15, wherein a speed of the coating is set within a range between 100 m/minute and 300 m/minute.

17. The method according to claim 3, wherein the dry-bulb temperature is gradually lowered as the support is conveyed from an entrance side of the plane air cushion drying step toward an exit side of the helical air cushion drying step.

18. The method according to claim 17, wherein a speed of the coating is set within a range between 100 m/minute and 300 m/minute.

\* \* \* \* \*